# EUROPEAN PATENT SPECIFICATION

(11) **EP 2 060 404 B1**
(45) Date of publication and mention of the grant of the patent: **13.04.2011**
(21) Application number: 08020088.4
(22) Date of filing: 18.11.2008
(51) Int. Cl.: B41M 5/52, B41N 1/24, B41M 5/00

(54) **Recording medium and producing method thereof, and inkjet recording method**
Aufzeichnungsmedium und Verfahren zu dessen Herstellung und Tintenstrahlaufzeichnungsverfahren
Support d'enregistrement et son procédé de production, et procédé d'enregistrement de jet d'encre

(30) Priority: 19.11.2007 JP 2007299921
(43) Date of publication of application: 20.05.2009
(73) Proprietor: FUJIFILM Corporation, Minato-ku Tokyo (JP)
(72) Inventor: Nakano, Ryoichi, Fujinomiya-shi, Shizuoka-ken (JP)
(74) Representative: HOFFMANN EITLE

(56) References cited:
- JP-A- 2005 105 443
- JP-A- 2007 136 812

## Description

### BACKGROUND OF THE INVENTION

### [Field of the invention]

The present invention relates to a recording medium and a producing method thereof and an inkjet recording method that uses the same.

### [Description of the related art]

An inkjet recording unit has a simple configuration and high quality image recording may be realized through inkjet recording using the inkjet recording unit. Ink used in inkjet recording is controlled such that a viscosity thereof is substantially from several mPa · s to 30 mPa·s such that it may be discharged from an inkjet head, and configured such that the surface tension may be substantially from 20 to 40 mN/m.

In order to control the viscosity of the ink to within this range, an ink solvent is usually contained in the ink at an amount of from 50% to 90% by mass. Examples of ink solvents include water, organic solvents, oils and photopolymerizing monomers. From the viewpoint of the environmental aptitude in particular, water is frequently used. Furthermore, in order to inhibit clogging due to drying of the ink solvent at a discharge nozzle of an inkjet head, a high boiling point solvent such as glycerin is generally used as an ink solvent.

However, when an ink solvent is present in a large amount in a ink drawn recording medium, image blurring and color mixing between colors are likely to be caused due to the abundancy of the ink solvent. Accordingly, inkjet-only paper (see Fig. 5) having a solvent absorption layer (ink-receiving layer) that absorbs the ink solvent and has a thickness of substantially 20 µm to 30 µm is used as a recording medium, thereby inhibiting image blurring and color mixing.

Furthermore, in the case of aqueous ink where water is used as an ink solvent, water permeates into the base paper at the time of recording to cause paper deformation such as curling. However, as shown in Fig. 5, when an inkjet-only paper 200 has a solvent absorbing layer 22 on a base paper 21, water is inhibited from permeating into the base paper; accordingly, the paper may be inhibited from deforming.

In this case in particular, when a graphical image having a high image density or having a high image area ratio is to be formed, an ink amount on a unit area on the recording medium increases, making it difficult for a solvent absorption layer to inhibit the ink solvent from permeating into the base paper. Accordingly, a water resistant paper covered with a resin layer that uses polyolefin (such as laminated paper) is generally used. (see, for example, Japanese Patent Application Laid-Open (JP-A) No. 2005-238829, Japanese Patent Application Laid-Open (JP-A) No. 2005-96285, Japanese Patent Application Laid-Open (JP-A) No. 2002-69890, and Japanese Patent Application Laid-Open (JP-A) No. 11-78224).

Moreover, an ink jet recording sheet for an oil-based ink has been proposed in which an ink penetration protection layer (lower layer) containing an aqueous emulsion resin, such as polyvinyl alcohol (PVA), and an ink holding layer (upper layer) containing a filler, such as silica or calcined kaolin, a water-soluble polymer, such as PVA, and an aqueous emulsion resin, such as styrene butadiene resin, are provided and the weight ratio of solids contained in the two layers is adjusted to be within a specific range (see, for example, Japanese Patent Application Laid-Open (JP-A) No. 3-234698).

Inkjet technology has been applied recently not only in the fields of office printers and home printers but also in commercial printing. In the field of the commercial printing, rather than paper that has a photograph-like surface that completely shuts out the ink solvent from permeating into a base paper, paper having printing texture similar to general printing paper is demanded. However, when a solvent absorbing layer that forms part of a recording medium becomes as thick as 20 to 30 µm, the surface glossiness, texture and hardness of the recording medium are limited; accordingly, inkjet technology in the commercial printing field is applied only to posters and ledger sheets printing in which the surface glossiness, texture and hardness of a recording medium may be limited.
Furthermore, owing to the adoption of the solvent absorbing layer and water resistant layer, the recording medium becomes expensive, and this is also a limiting factor.

### SUMMARY OF THE INVENTION

Various recording media have been developed in which penetration of an ink solvent into a base paper and the like occurring in connection with image recording are suppressed by devising the composition of each layer provided on the base paper. However, a recording medium in which the development of curl, image bleeding, and mixing of colors are prevented and peeling of ink is taken into consideration has not been found.

The present invention aims to provide a recording medium which can form a high quality image in which the development of curl, image blur, and mixing of colors occurring in connection with image recording are prevented and separation of ink is difficult to occur; a method of producing the recording medium; and an ink jet recording method which allows formation of a high quality image at low cost and at high speed. A first aspect of the present invention provides a recording medium, (100) according to claim 1, comprising: a base paper (11), a first layer (12) containing a binder, and a second layer (13) containing kaolin and polyvinyl alcohol, the base paper (11), the first layer (12), and the second layer (13) being successively laminated, wherein a Cobb water absorption degree during a contact time of 120 seconds by a water absorption test according to JIS P8140 on the surface of the first layer (12) formed on the base paper (11) on which the first layer(12) has been formed is 2.0 g/m² or less; and the water absorption amount during a contact time of 0.5 second by the Bristow method on the surface of the second layer (13) is from 2 mL/m² to 8 mL/m².

A second aspect of the present invention provides a method of producing of the recording medium (100) according to the first aspect, the method comprising: forming a first layer (12) on a base paper (11) by applying a film formation liquid containing a thermoplastic resin particle, and heating at a temperature range equal to or higher than the minimum film forming temperature of the thermoplastic resin particle; and forming a second layer (13) on the first layer (12) by applying a film formation liquid containing kaolin and polyvinyl alcohol to the first layer (12).

A third aspect of the present invention provides an ink jet recording method, comprising: applying a treatment liquid containing an acid substance to the recording medium (100) according to the first aspect of the invention; applying ink to the recording medium (100) to which the treatment liquid has been applied, and performing ink drawing according to predetermined image data; and drying and removing an ink solvent in the recording medium (100) on which ink drawing has been performed.

### BRIEF DESCRIPTION OF THE DRAWINGS

Exemplary aspects of the invention will be described in detail based on the following figures, wherein:
Fig. 1 is a schematic constitutional diagram showing a configuration example of a recording medium of the invention.
Fig. 2 is an explanatory diagram for explaining an example of an inkjet recording method involving a first aspect that uses a recording medium of the invention.
Fig. 3 is an explanatory diagram for explaining an example of an inkjet recording method involving a second aspect that uses a recording medium of the invention.
Fig. 4 is a diagram for explaining a scanning line of a head in which a test liquid is filled in the Bristow method.
Fig. 5 is a schematic constitutional diagram showing a structure of an existing recording medium.

### DETAILED DESCRIPTION

Exemplary embodiments of the invention are described in detail hereinafter.

An object of the present invention is to solve the above-described problems, and the problems are solved by the invention as described below.

A first exemplary embodiment of the invention is a recording medium (100), comprising:
a base paper (11), a first layer (12) containing a binder, and a second layer (13) containing kaolin and polyvinyl alcohol, the base paper (11), the first layer (12), and the second layer (13) being successively laminated, wherein a Cobb water absorption degree during a contact time of 120 seconds by a water absorption test according to JIS P8140 on the surface of the first layer (12) formed on the base paper (11) on which the first layer(12) has been formed is 2.0 g/m² or less; and the water absorption amount during a contact time of 0.5 second by the Bristow method on the surface of the second layer (13) is from 2 mL/m² to 8 mL/m²_{,}
wherein the kaolin has a whiteness degree of more than 87 and the composition ratio (volume ratio) of kaolin having a particle diameter of 2 µm or less is 75% or more with respect to a total volume of kaolin, and wherein the degree of polymerization of the polyvinyl alcohol is 1,500 or more.

A second exemplary embodiment of the invention is the recording medium (100) according to the first exemplary embodiment, wherein the content of the kaolin in the second layer (13) is from 75% by mass to 99% by mass with respect to the total solid content of the second layer (13).

A third exemplary embodiment of the invention is the recording medium (100) according to the first or second exemplary embodiments, wherein the binder in the first layer (12) contains a thermoplastic resin.

A fourth exemplary embodiment of the invention is the recording medium (100) according to the third exemplary embodiment, wherein the thermoplastic resin is at least one selected from the group consisting of polyester urethane latex and acrylic silicone latex.

A fifth exemplary embodiment of the invention is the recording medium (100) according to any one of the first to fourth exemplary embodiments, wherein the first layer (12) further contains a white pigment.

A sixth exemplary embodiment of the invention is the recording medium (100) according to fifth exemplary embodiment, wherein the white pigment is kaolin.

A seventh exemplary embodiment of the invention is a producing method of a recording medium for producing the recording medium (100) according to any one of the third to sixth exemplary embodiment, the method comprising: forming a first layer (12) on a base paper (11) by applying a film formation liquid containing a thermoplastic resin particle, and heating at a temperature range equal to or higher than the minimum film forming temperature of the thermoplastic resin particle; and forming a second layer (13) on the first layer (12) by applying a film formation liquid containing kaolin and polyvinyl alcohol to the first layer (12).

An eigth exemplary embodiment of the invention is an ink jet recording method, comprising: applying ink to the recording medium (100) of any one of the first to sixth exemplary embodiment, and performing ink drawing according to predetermined image data, and drying and removing an ink solvent in the recording medium (100) on which ink drawing has been performed.

A ninth exemplary, embodiment of the invention is an ink jet recording method, comprising: applying a treatment liquid containing an acid substance to the recording medium (100) of any one of the first to sixth exemplary embodiment; applying ink to the recording medium (100) to which the treatment liquid has been applied, and performing ink drawing according to predetermined image data; and drying and removing an ink solvent in the recording medium (100) on which ink drawing has been performed.

In what follows, a recording medium of the invention and producing method thereof and an inkjet recording method that uses the recording medium will be described in detail.

### <Recording Medium>

A recording medium of the invention is formed by including a base paper, a first layer and a second layer sequentially disposed in this order from the base paper side, and, as needs arise, appropriately selected other layer. A recording medium of the invention, like, for instance, a recording medium 100 shown in Fig. 1, is constituted by disposing a high-quality paper 11 as a base paper, a solvent-blocking layer 12 as a first layer formed on the high-quality paper 11 and a coated layer 13 as a second layer formed on the solvent-blocking layer 12. Furthermore, the recording medium may be either a sheet paper or a roll paper.

### (Base Paper)

The base paper is not particularly restricted and may be appropriately selected from known ones depending on the object.

As pulp that is used as a raw material of a base paper, from the viewpoints of simultaneously improving the surface smoothness, stiffness and dimensional stability (curling property) of the base paper with balance to a high level, leaf bleached kraft pulp (LBKP) is desirable. Furthermore, needle bleached kraft pulp (NBKP) and leaf bleached sulfite pulp (LBSP) may be used as well.

When the pulp is digested, a beater or a refiner may be used. In a pulp slurry (hereinafter, in some cases, referred to as "pulp paper stock") obtained after the pulp is digested, as needs arise, various kinds of additives such as a filler, a dry paper strengthening agent, a sizing agent, a wet paper strengthening agent, a fixing agent, a pH regulating agent and other chemicals are added.

Examples of fillers include calcium carbonate, clay, kaolin, white earth, talc, titanium oxide, diatom earth, barium sulfate, aluminum hydroxide and magnesium hydroxide.

Examples of the dry paper strengthening agents include cationized starch, cationized polyacrylamide, anionized polyacrylamide, amphoteric polyacrylamide and carboxy-modified polyvinyl alcohol.

Examples of the sizing agents include fatty acid salt, rosin, rosin-derivatives such as maleinized rosin, paraffin wax, alkyl ketene dimer, alkenyl succinate anhydride (ASA) and epoxidized fatty acid amide.

Examples of the wet paper strengthening agents include polyaminepolyamide epichlorohydrine, a melamine resin, a urea resin and an epoxidized polyamide resin.

Examples of the fixing agents include multi-valent metal salts such as aluminum sulfate or aluminum chloride and cationized polymers such as cationized starch.

Examples of the pH regulating agents include sodium hydroxide and sodium carbonate.

Examples of the other chemicals include a defoaming agent, a dye, a slime control agent and a fluorescent brightener.

Furthermore, to the pulp paper stock, as needs arise, a softener may be added as well. The softener is described in, for instance, "Sin Kamikakou Binran (New Paper Processing Handbook)" (edited by Siyaku Times Cho.,), 554 to 555 (1980).

In a treatment solution used in surface sizing, for instance, an aqueous polymer, a sizing agent, a water resistant material, a pigment, a pH adjusting agent, a dye and a fluorescent brightener may be contained.

Examples of the aqueous polymers include cationized starch, polyvinyl alcohol, carboxy-modulated polyvinyl alcohol, carboxymethylcellulose, hydroxyethylcellulose, cellulose sulfate, gelatin, casein, sodium polyacrylate, sodium salt of styrene-maleic anhydride copolymer and sodium polystyrene sulfonate.

Examples of the sizing agents include petroleum resin emulsion, ammonium salt of styrene-maleic anhydride copolymer alkyl ester, rosin, higher fatty acid salt, alkyl ketene dimer (AKD) and epoxidized fatty acid amide.

Examples of the water resistant materials include latex emulsions of styrene-butadiene copolymer, ethylene-vinyl acetate copolymer, polyethylene or vinylidene chloride copolymer and polyamidepolyamine epichlorhydrine.

Examples of the pigments include calcium carbonate, clay, kaolin, talc, barium sulfate and titanium oxide.

Examples of the pH adjusting agents include hydrochloric acid, sodium hydroxide and sodium carbonate.

Examples of materials of base papers may include, other than the above-mentioned natural pulps, synthetic pulp paper, mixed paper of natural pulp and synthetic pulp and various kinds of combination papers.

A thickness of the base paper is preferably from 30 to 500 µm, more preferably from 50 to 300 µm and still more preferably from 70 to 200 µm.

### (First Layer)

On the base paper of a recording medium of the invention, a first layer is disposed. After the first layer has been disposed, an ink solvent is suppressed from permeating into the base paper. For instance, as a paper provided with a solvent-blocking layer, one where a coating layer mainly made of a polyethylene resin is disposed on a surface of the base paper is known. However, the paper where the solvent-blocking layer is disposed to impart the water resistance is, although substantially complete in the water-blocking effect, not necessarily satisfying in the texture as the paper.

The first layer includes at least a binder and the Cobb's water absorbency of a surface of the first layer of the base paper provided with the first layer is set at 2.0 g/m² or less during a contact time of 120 sec according to the water absorbency test according to JIS P8140. As far as the Cobb's water absorbency is within the range, without particular restriction, the first layer, depending on the object, may be appropriately selected from known ones.

Furthermore, the first layer may be constituted, as needs arise, by use of, other than the binder, other components such as a crosslinking agent and a white pigment.

As the first layer of the present invention, from the viewpoint of suppressing penetration of an ink solvent and obtaining favorable surface properties, a preferable layer is, for example, a layer which contains, as a binder, a thermoplastic resin (preferably latex, and more preferably polyester urethane latex or acrylic silicone latex) and contains Kaolin as a white pigment and in which a mass ratio x/y of the mass (solid content) x of thermoplastic resin and the mass y of kaolin is adjusted to from 1 to 30 or a layer containing, in addition to the above-mentioned components, a cross linking agent selected from epoxy compounds, compounds containing an active methylene group, cyanuric chloride, formaldehyde, and carbodiimide.

### -Binder-

The first layer includes at least one kind of binders. The binder is used not only to disperse but also to improve the strength of a coated film.

Examples of the binders include polyvinyl alcohols (including modified polyvinyl alcohols such as acetoacetyl-modified, carboxyl-modified, itaconic-modified, maleic-modified, silica-modified or amino group-modified one), methylcellulose, carboxy methylcellulose, starches (including modified starches), gelatin, rubber Arabic, casein, a styrene-maleic anhydride copolymer hydrolysate, polyacrylamide and saponified vinyl acetate-acrylic acid copolymer. Furthermore, latex type thermoplastic resins of synthetic polymers such as styrene-butadiene copolymer, vinyl acetate copolymer, acrylonitrile-butadiene copolymer, methyl.acrylate-butadiene copolymer or polyvinylidene chloride.

Examples of the polyvinyl alcohols include polyvinyl alcohols obtained by saponifying a lower alcohol solution of polyvinyl acetate and derivatives thereof and ones obtained by saponifying a copolymer between a monomer copolymerizing with vinyl acetate and vinyl acetate. Herein, examples of the monomers capable of copolymerizing with vinyl acetate include unsaturated carboxylic acid such as (anhydrous) maleic acid, fumaric acid, crotonic acid, itaconic acid, (meth)acrylic acid or an esters thereof; α-olefin such as ethylene or propylene; olefin sulfonic acid such as (meth)allyl sulfonic acid, ethylene sulfonic acid or sulfonic acid alkylmaleate; an alkali salt of olefin sulfonic acid such as sodium (meth)allylsulfonate, sodium ethylene sulfonate, sodium sulfonate alkyl (meth)acrylate, sodium sulfonate (monoalkyl malate) or sodium disulfonate alkyl malate; an amide group-containing monomer such as N-methylolacrylamide or an alkali salt of acrylamide alkylsulfonate; and a N-vinyl pyrolidone derivative.

Among polyvinyl alcohols, acetoacetyl modified polyvinyl alcohol can generally be produced by adding liquid or gaseous diketene to a solution, dispersion liquid, or powder of the polyvinyl alcohol for reaction. The degree of acetylation of acetoacetyl modified polyvinyl alcohol can be suitably determined according to the target quality, and is preferably from 0.1% by mol to 20% by mol, and more preferably from 0. 5% by mol to 10% by mol.

Examples of the binders further include, in addition to general-purpose thermoplastic polymers such as polyolefins such as homopolymers of α-olefin such as polyethylene, polypropylene or polyvinyl chloride or mixtures thereof; polyamides and polyimides; and polyesters such as polyethylene terephthalate, known thermoplastic resins and latexes thereof such as homopolymers made of α-methylene fatty acid monocarboxylic acid esters such as methyl (meth)acrylate, ethyl (meth)acrylate, butyl (meth)acrylate, dodecyl (meth)acrylate, octyl (meth)acrylate or phenyl (meth)acrylate; styrenes such as styrene, chlorostyrene or vinyl styrene; vinyl esters such as vinyl acetate, vinyl propionate, vinyl succinate or vinyl butyrate; vinyl ethers such as vinyl methyl ether, vinyl ethyl ether or vinyl butyl ether; or vinyl ketones such as vinyl methyl ketone, vinyl hexyl ketone or vinyl isopropyl ketone, or as arbitrary copolymers containing the constitutional units.

Among the above, in terms of water barrier properties, a thermoplastic resin is preferable and latex is more preferable. Examples of latex include latex of thermoplastic resin, such as acrylic latex, acrylic silicone latex, acrylic epoxy latex, acrylic styrene latex, acrylic urethane latex, styrene-butadiene latex, acrylonitrile-butadiene latex, polyester urethane latex, and vinyl acetate latex. In particular, polyester urethane latex and acrylic silicone latex are preferable from the viewpoint that effects of suppressing ink solvent permeability and cockling are high and both economical efficiency and production suitability are given.

A molecular weight of the latex, by number average molecular weight, is preferably from 3,000 to 1,000,000 and particularly preferably substantially from 5,000 to 100,000. The molecular weight, when it is 3,000 or more, allows securing the mechanical strength of the first layer and, when it is 1,000,000 or less, is advantageous from the production aptitudes such as dispersion stability and viscosity.

Specifically, as the acrylic latex, commercially available products such as water dispersive latexes described below are used. That is, preferable examples of the acrylic resins include "CEBIAN A4635, 46583 and 4601" (trade name, manufactured by Daicel Chemical Industries, Ltd.) and "NIPOL Lx811, 814, 820, 821 and 857" (trade name, manufactured by ZEON CORPORATION.). In particular, acryl emulsions of acryl silicone latexes described in JP-A Nos. 10-264511, 2000-43409, 2000-343811 and 2002-120452 (commercially available products include AQUABRID-series UM7760, UM7761 and UM4901, AQUABRID 903, AQUABRID ASi-86, AQUABRID ASi-89, AQUABRID ASi-91, AQUABRID ASi-753, AQUABRID ASi-4635, AQUABRID ASi-4901, AQUABRID MSi-04S, AQUABRID AU-124, AQUABRID AU-131, AQUABRID AEA-61, AQUABRID AEC-69 and AQUABRID AEC-162) are preferably used.

Moreover, examples of polyester urethane latex include commercially-available items, such as HYDRAN AP series, manufactured by DIC Corporation (e.g., HYDRAN AP-20, HYDRAN AP-30, HYDRAN AP-30F, HYDRAN AP-40(F), HYDRAN AP-50LM, HYDRAN APX-101H, HYDRAN Apex-110, and HYDRAN Apex-501).

It should be noted that it is preferable to select at least one member from the above-mentioned thermoplastic resins for use. The above-mentioned thermoplastic resins may be used singly or in combination of two or more.

The glass transition temperature (Tg) of the thermoplastic resin contained in the first layer is preferably 5°C to 70°C and particularly preferably 15°C to 50°C. When the Tg is in the range in particular, a film-forming solution (such as coating solution) for forming a first layer is inhibited from causing a problem such as skinning to be easy to handle in production. Furthermore, without causing problems such that the Tg is too high to be able to obtain desired glossiness unless a calender temperature is set rather high and adhesion to a surface of a metal roll tends to occur to adversely affect on a surface state, high glossiness and high planarity are readily obtained.

Furthermore, the minimum film-forming temperature of the thermoplastic resin (preferably latex resin fine particles) is preferably from 20 to 60°C and more preferably from 25 to 50°C. When the minimum film-forming temperature region capable of forming a film when a film is formed is within the range, the film-forming solution for forming the first layer (such as coating solution) is inhibited from a problem such as the skinning to be easy to handle in the production, and, when the second layer is formed, the permeation is suppressed to be excellent in a state of the coated surface of the formed second layer; accordingly, a layer having the microporosity sufficient for speedily transmitting an ink solvent is formed. Only by coating the solution (such as coating solution), excellent glossiness is not necessarily provided. However, when soft calender treatment is applied thereafter, a highly glossy layer having the microporosity is obtained.

A content of the binder (preferably thermoplastic resin) in the first layer is, relative to a total solid content of the first layer, preferably from 15 to 95% by mass and more preferably from 30 to 90% by mass. In the case where the content is within the range in particular, when the _ calender process is applied, the glossiness and planarity are excellent, the permeability of the ink solvent is obtained and the blurring with time is more effectively inhibited from occurring.

Furthermore, in the first layer, as needs arise, depending on the kind of the binder, an appropriate crosslinking agent of the binder may be added.

### -Cobb's Water Absorbency-

In the invention, the Cobb's water absorbency measured according to the water absorbency test based on JIS P8140 from a first layer side of a base paper on which the first layer is disposed for 120 sec is set at 2.0 g/m² or less. When the Cobb's water absorbency is 2.0 g/m² or less, the base paper provided with the first layer has mild permeability to be able to delay absorption when a liquid such as ink is provided and reduce the degree of occurrence of curling.

Furthermore, the Cobb's water absorbency is preferred to be 1.0 g/m² or less. Still furthermore, the minimum value of the Cobb's water absorbency is desirably 0.2 g/m².

The Cobb's water absorbency is measured according to a water absorbency test based on JIS P8140 and an amount of absorbed water measured when water is brought into contact for a definite time from one surface of the base paper, specifically, a surface of the first layer of the base paper on which the first layer is disposed. In the invention, a contact time is set at 120 sec.

In the first layer, other than the components, other components such as a white pigment, a film hardening agent and a layered inorganic compound may be used.

### -White Pigment-

Examples of the white pigments include titanium oxide, barium sulfate, barium carbonate, calcium carbonate, lithopone, alumina white, zinc oxide, silica antimony trioxide, titanium phosphate, aluminum hydroxide, kaolin, clay, talc, magnesium oxide and magnesium hydroxide.

Moreover, kaolin other than calcined kaolin is particularly preferable in terms of water interception. Examples of such kaolin include procucts of Imerys Minerals Japan K.K., such as Astra-Plus, Contour 1500, Contour Xtreme, Capim DG, Capim NP, Capim CC, Astra-Sheen, Astra-Gross, Astra-Cote, Beta-bright, Astra-Graze, Premier LX, Premier K.C.S., Astra-Plate, and XP03-8390; products of Shiraishi Calcium Kaisha, Ltd., such as Kaogloss 90, Kaobright 90, Kaolux HS; Kaowhite S, Kaowhite, Kaowhite C, Kaofine, Kaogloss, and Kaobright; products of TAKEHARA KAGAKU KOGYO CO., LTD., such as Union clay RC-1, NN kaolin clay, SPMA clay, kaolin clay 5M, Hardsil, ST kaolin clay, Katarupo, and No. 5 clay; products of J.M.Huber Corporation, such as Huber 35, Huber 35B, Huber 80, Huber 80B, Huber 90, Huber 90B, Huber HG-90, Huber TEK-2001, Polygloss 90, Polyplate P, Polyplate P01, Polyplate HMT, Lithosperse 7005CS, Zeolex 94HP, Zeolex 323, and Zeolex 325.

In the case where the white pigment is contained in the first layer, when a calender process is applied after the first layer is formed, the first layer is inhibited from sticking to the calender.

As the particle size of the white pigment, particles of 2.0 µm or less are preferably contained 75% or more by volume base. When the particle size is in the range, the whiteness and glossiness become excellent.

Furthermore, the specific surface area of the white pigment due to the BET method is preferred to be less than 100 m²/g. When the white pigment having the specific surface area in the range is contained, when the second layer is coated and formed, the coating solution is inhibited from permeating; accordingly, the ink absorptivity of the second layer is heightened.

The BET method is one of surface area measurement methods of powder due to a gas phase adsorption method and a method where, from an adsorption isotherm, a total surface area that 1 g of sample has, that is, specific surface area is obtained. Usually, a method where, as an adsorption gas, nitrogen gas is used and an absorption amount is measured from a variation of pressure or volume of a gas to be adsorbed is general. As well-known one that expresses an isotherm of multimolecular adsorption, there is an equation of Brunauer, Emmett and Teller (BET equation). Based on the equation, an adsorption amount is obtained, followed by multiplying an area that one absorption molecule occupies on a surface to obtain a surface area.

The white pigments may be used singularly or in a combination of two or more kinds thereof.

A content of the white pigment in the first layer is, though different dependent on the kind of the white pigment, the kind of the thermoplastic resin and the layer thickness, relative to a mass (solid content) of the binder, usually desirably substantially in the range of 5 to 200% by mass.

### -Hardener-

The first layer of the invention may include a hardener to harden the binder. Examples of the hardeners include aldehyde compounds, 2,3-dihydroxy-1,4-dioxane and derivatives thereof and compounds that have two or more of vinyl groups adjacent to a substitution group of which Hammett's substituent constant σₚ is positive in a single molecule.

When the first layer contains the hardener, without thickening the film-forming solution of the first layer, the water resistance of the recording medium may be improved. Thereby, the coating stability of the film-forming solution of the first layer is improved and thereby the water resistance of the resulting recording medium as well is improved.

Examples of substitutional groups of which Hammett's substituent constant σₚ is positive include a CF₃ group (σₚ value: 0.54), a CN group (σₚ value: 0.66), a COCH₃ group (σₚ value: 0.50), a COOH group (σₚ value: 0.45), a COOR (R expresses an alkyl group) group (σₚ value: 0.45), a NO₂ group (σₚ value: 0.78), a OCOCH₃ group (σₚ value: 0.31), a SH group (σₚ value: 0.15), a SOCH₃ group (σₚ value: 0.49), a SO₂CH₃ group (σₚ value: 0.72), a SO₂NH₂ group (σₚ value: 0.57), a SCOCH₃ (σₚ value: 0.44), a F group (σₚ value: 0.06), a Cl group (σₚ value: 0.23), a Br group (σₚ value: 0.23), a I group (σₚ value: 0.18), a I0₂ group (σₚ value: 0.76), a N⁺(CH₃)₂ group (σₚ value: 0.82), and a S⁺(CH₃)₂ group (σₚ value: 0.90).

Examples of the compounds that have two or more of vinyl groups adjacent to a substitution group of which Hammett's substituent constant σₚ is positive in a single molecule include, in addition to 2-ethylenesulfonyl-N-[2-(2-ethylenesulfonyl-acetylamino)-ethyl]acetamide, bis-2-vinylsulfonylethyl ether, bisacryloylimide, N-N'-diacryloyl urea, 1,1-bisvinylsulfone ethane and ethylene-bis-acrylamide, diacrylate and dimethacrylate compound expressed by formulae below, among these 2-ethylenesulfonyl-N-[2-(2-ethylenesulfonyl-acetylamino)-ethyl]acetamide being particularly preferred.

A content of the hardener in the first layer is, relative to a solid content of the binder, preferably 0.1% by mass or more and 30% by mass or less and more preferably 0.5% by mass or more and 10% by mass or less. When the content of the hardener is within the range, the film-forming solution for the first layer is not thickened and the water resistance of the recording medium may be improved.

### -Layered Inorganic Compound-

The first layer may further contain a layered inorganic compound. The layered inorganic compound is preferred to be a swelling inorganic layered compound and examples thereof include swelling clayey ores such as bentonite, hectorite, saponite, biederite, nontronite, stevensite, beidelite or montmorillonite, swelling synthetic mica and swelling synthetic smectite. The swelling inorganic layered compound has a stacked structure made of unit crystal lattice layers having a thickness from 1 to 1.5 nm and is very large in the metallic atom substitution within a lattice than other clayey ores; accordingly, a lattice layer causes positive charge deficiency and, in order to compensate the deficiency, positive ions such as Na⁺, Ca²⁺ or Mg²⁺ are adsorbed between layers. The positive ion interposing between the layers is called an exchangeable positive ion and is exchanged by various positive ions. In particular when the interlayer positive ion is Li⁺ or Na⁺, owing to small ionic radius, bonding between layered crystal lattices is weak to be largely swollen by water. When shearing force is applied in this state, the layered inorganic compound is readily cleaved to form stable sol in water. Bentonite and water swellable synthetic mica are preferred because this tendency is strong. The water swellable synthetic mica is particularly preferred.

Examples of the water swellable synthetic micas include sodium tetrasilicic mica NaMg_{2.5}(Si₄O₁₀)F₂Na, lithium teniolite (NaLi)Mg₂(Si₄O₁₀)F₂Na or lithium hectolite (NaLi)/3Mg₂/3Li_{1/3}SiO₄O₁₀)F2.

As to the size of the water swellable mica, it is preferable that a thickness is from 1 to 50 nm and a face size is from 1 to 20 µm. In order to control the diffusion, the thinner the thickness is, the better, and a plain size is better larger within a range that does not deteriorate the smoothness and transparency of a coated surface. Accordingly, the aspect ratio is preferably 100 or more, more preferably 200 or more and particularly preferably 500 or more.

When the water swellable synthetic mica is used, a mass ratio x/y of a mass (solid content) x of a binder in the first layer to a mass y of water swellable synthetic mica is preferably in the range of 1 or more and 30 or less and more preferably in the range of 5 or more and 15 or less. When the mass ratio is within the range, oxygen permeation and blister generation are effectively suppressed.

In the first layer, a known additive such as an anti-oxidant as well may be added.

A thickness of the first layer is preferably in the range of 1 to 30 µm and more preferably in the range of 5 to 20 µm. When the thickness of the first layer is within the range, the surface glossiness when the calender treatment is applied later is improved, the whiteness is obtained with a slight amount of the white pigment and the handling property such as folding aptitude is made same as that of a coat paper or an art paper.

### (Second layer)

The recording medium of the present invention further has a second layer on the first layer on a base paper.

The second layer contains at least kaolin and polyvinyl alcohol both as specified in claim 1. The amount of water absorption during a contact time of 0.5 second of the surface of the second layer by Bristow method is adjusted to be within the range of from 2 mL/m² to 8 mL/m². There is no limitation on the second layer insofar as the amount of water absorption is within the range. The second layer can be suitably selected known substances according to the purpose.

Moreover, the second layer can be formed further using another component, such as a thermoplastic resin, as required.

The second layer in the invention is preferred to be, for instance, a layer that further includes a thermoplastic resin, a layer that further contains a thermoplastic resin of 10 to 60 parts by solid mass to 100 parts by solid mass of the kaolin or a layer where the pH of a layer surface is 4 or less.

### -Kaolin-

The second layer contains at least one type of kaolin. By containing kaolin, ink (especially, a pigment in ink) can be kept in the second layer, and the degree of whiteness of the ground is also increased.

As kaolin contained in the second layer, kaolin other than calcined kaolin is preferable in terms of prevention of image blur, mixing of colors, and film strength. Examples of such kaolin include products of Imerys Minerals Japan K.K., such as Astra-Plus, Contour 1500, Contour Xtreme, Capim DG, Capim NP, Capim CC, Astra-Sheen, Astra-Gross, Astra-Cote, Beta-bright, Astra-Graze, Premier LX, Premier K.C.S., Astra-Plate, and XP03-8390; products of Shiraishi Calcium Kaisha, Ltd., such as Kaogloss 90, Kaobright 90, Kaolux HS, Kaowhite S, Kaowhite, Kaowhite C, Kaofine, Kaogloss, and Kaobright; products of TAKEHARA.KAGAKU KOGYO CO., LTD., such as Union clay-RC-1, NN kaolin clay, SPMA clay, kaolin clay 5M, Hardsil, ST kaolin clay, Katarupo, and No. 5 clay; products of J.M.Huber Corporation, such as Huber 35, Huber 35B, Huber 80, Huber 80B, Huber9 0, Huber 90B, Huber HG-90, Huber TEK-2001, Polygloss 90, Polyplate P, Polyplate P01, Polyplate HMT, Lithosperse 7005CS, Zeolex 94HP, Zeolex 323, and Zeolex 325.

kaolin having a whiteness degree exceeding 87 is mandatory, and kaolin having a whiteness degree of 90 or more is more preferable. When the whiteness degree of kaolin exceeds 87, an image-receiving paper can be effectively prevented from coloring, and thus high quality feeling of paper can be maintained over a long period of time.

Moreover, as the particle diameter of kaolin contained in the second layer, the composition ratio (volume ratio) of kaolin having a particle diameter of 2 µm or lower is 75% or more, and more preferably 80% or more. When the proportion of kaolin having a particle diameter of 2 µm or lower is 75% or more, the gloss is high and high quality feeling of paper can be produced.

A content of the kaolin in the second layer is, to a total solid content of the second layer, preferably from 75 to 99% by mass and more preferably from 80 to 96% by mass.

In the second layer, in order not to impair the effects of the present invention, white pigments other than kaolin, can be blended. Examples of such white pigments include titanium oxide, barium sulfate, barium carbonate, calcium carbonate, lithopone, alumina white, zinc oxide, silica antimony trioxide, titanium phosphorate, aluminum hydroxide, clay, talc, magnesium oxide, and magnesium hydroxide. When image formation is carried out by using the recording medium of the present invention according to the first or second ink jet recording method of the present invention described below, i.e., when ink drawing is performed while adjusting the pH of the layer surface of the second layer to the acidic side (preferably 4 or lower) or using a treatment liquid containing an acid substance mentioned below, the content of calcium carbonate is preferably 1% by mass or lower based on the total pigment content in the second layer from the viewpoint that image blur and mixing of colors at the time of performing ink drawing are prevented, and it is more preferable that no calcium carbonate is contained.

### - Polyvinyl alcohol-

The second layer contains at least one type of polyvinyl alcohol having a degree of polymerisation of 1500 or more.

Polyvinyl alcohol obtained by saponifying a lower alcohol solution of polyvinyl acetate and derivatives thereof and saponified substances of a copolymer of a monomer capable of being copolymerized with vinyl acetate and vinyl acetate can be used. Here, examples of the monomer capable of being copolymerized with vinyl acetate include unsaturated carboxylic acid and esters thereof, such as (anhydrous) maleic acid, fumaric acid, crotonic acid, itaconic acid, and (meth)acrylic acid; α-olefins, such as ethylene and propylene; olefin sulfonic acids, such as (meth) allylsulfonic acid, ethylene sulfonic acid, and sulfonic acid malate; olefin sulfonic acid alkali salts, such as (meth) allylsulfonic acid soda, ethylene sulfonic acid soda, sulfonic acid soda (meth) acrylate, sulfonic acid soda (monoalkyl malate), and disulfonic acid soda alkyl malate; amide group-containing monomers, such as N-methylolacrylamide and acrylamide alkyl sulfonic acid alkali salt; and N-vinyl-pyrrolidone derivatives.

For example, modified polyvinyl alcohols, such as acetyl modified polyvinyl alcohol, carboxy modified polyvinyl alcohol, itaconic acid modified polyvinyl alcohol, maleic acid modified polyvinyl alcohol, silica modified polyvinyl alcohol, and amino group modified polyvinyl alcohol, can also be employed.

For example, acetoacetyl modified polyvinyl alcohol has sufficient oxygen permeation inhibition and high S-S properties. The S-S properties as used herein refer to the absorption amount of tension energy (toughness) indicated as stress-elongation until a film is fractured. Therefore, the first layer freely expands relative to treatment requiring heating, and thus no cracking occurs and a blister is difficult to form.

It should be noted that the modification ratio of modified polyvinyl alcohol is preferably from 0.05% by mol to 20% by mol, and more preferably from 0.05% by mol to 15% by mol, from the viewpoint of achieving water resistance through a reaction with a hardener and the stability in an aqueous solution.

The degree of polymerization of polyvinyl alcohol contained in the second layer is 1,500 or more, and more preferably 2,000 or more. When the degree of polymerization is 1,500 or more, effects of suppressing the formation of cracking and separation of ink in a low moisture environment (e.g., 20°C, 10%) are increased. This is considered to result from that strength and elongation at the time of fracture can be remarkably increased by increasing the degree of polymerization to be as high as 1,500 or more. Moreover, when the degree of polymerization is increased, the viscosity of a coating liquid increases and the coated surface state decreases. However, the disadvantage is compensated by reducing the concentration of the coating liquid and the proportion of water dispersible mica.

The degree of saponification of polyvinyl alcohol is not limited, and is preferably 85% or more, and more preferably from 87% to 99%. When the degree of saponification of polyvinyl alcohol is 85% or more, a waterproof effect can be remarkably increased.

The mass ratio a/b of the mass a of polyvinyl alcohol (solid content) contained in the second layer to the mass b of kaolin contained in the second layer is preferably from 2:1 to 30:1, more preferably from 3:1 to 25:1, and particularly preferably from 5:1 to 20:1. When the mass ratio a/b of polyvinyl alcohol to kaolin is from 2:1 to 30:1, oxygen permeation and the formation a blister are suppressed and also favorable surface properties are achieved, whereby separation of ink can be effectively suppressed.

### -Thermoplastic resin-

The second layer may contain other components, such as thermoplastic resin, in addition to the above-mentioned components.

There is no limitation on the thermoplastic resin. For example, the thermoplastic resins as previously mentioned in the description of the first layer can be similarly used.

### -Amount of Water Absorption according to Bristow Method-

In the invention, an amount of water absorption during a contact time of 0.5 sec in a surface of the second layer due to the Bristow method is set at 2 mL/m² or more and 8 mL/M² or less. When the amount of water absorption is 2 to 8 mL/m², the second layer is mildly permeative to be able to retard liquid absorption at a surface where a liquid such as ink is imparted to suppress the degree of curling and to inhibit the color mixing between colors from occurring. In order to inhibit the blurring or color mixing between colors from occurring, as will be described below, it is particularly effective that the pH of a layer surface of the second layer is controlled acidic (in particular, 4 or less in the pH) or a treatment solution containing an acidic substance described below is used together with ink.

The amount of water absorption in the second layer is more preferable, from the reason same as that mentioned above, to be 2 mL/m² or more and 4 mL/m² or less.

The Bristow method is a method used as a method of measuring an amount of liquid absorption during a short time and is adopted also in Japan Technical Association of the Pulp and Paper Industry (J'TAPPI). The detail of the test method will be referenced to J. TAPPI PAPER, Pulp Test Method No. 51 to 87 "Liquid Absorbency Test Method of Paper and Paperboard" (Bristow Method) and TAPPI JOURNAL 41(8), 57 to 61 (1987). Herein, by use of a test unit (Bristow test machine) described above, a contact time is set at 0.5 sec to measure and, at the time of measurement, a slit width of a head box of the Bristow test unit is controlled adapted to the surface tension of ink. Furthermore, the ink strike-through is eliminated from calculation.

### -pH-

In the second layer, the pH of the layer surface is preferably controlled to 4 or less, thereby, the imparted ink is coagulated to result in an improvement in ink fixing. That is, in the case of ink that contains for instance a pigment as a coloring component, when the ink strikes the second layer, the pigment is coagulated owing to a variation of the pH to be able to inhibit the ink from blurring with time and the color mixing between colors from occurring.

Examples of compounds that make a surface of the second layer acidic include compounds that have a phosphoric acid group, a phosphonic acid group, a phosphinic acid group, a sulfuric acid group, a sulfonic acid group, a sulfinic acid group or a carboxylic acid group or a group derived from the salt thereof, a compound having a phosphoric acid group or a carboxylic acid group being preferably used.

Examples of compounds that have a phosphoric acid group include phosphoric acid, polyphosphoric acid or derivatives of compounds thereof, or salts thereof. Examples of compounds that have a carboxylic acid group include compounds that have a furan, pyrrole, pyrroline, pyrolidone, pyrone, pyrrole, thiophene, indole, pyridine or quinoline structure and further have a carboxyl group as a functional group such as pyrolidone carboxylic acid, pyrone carboxylic acid, pyrrole carboxylic acid, furan carboxylic acid, pyridine carboxylic acid, coumaric acid, thiophene carboxylic acid, nicotinic acid, or derivatives thereof, or salts thereof.

When one of the compounds is added to a film-forming solution for the second layer, the pH may be controlled to 4 or less. An addition amount may well be appropriately selected so that the pH may be 4 or less.

The pH is measured according to an A method (coating method) of methods for measuring the film surface pH, which is determined by Japan Technical Association of the Pulp and Paper Industry (J. TAPPI), and a method that corresponds to, for instance, the A method and uses a paper surface pH measurement set "Form MPC" (trade name, manufactured by Kyoritsu Chemical-Check Lab., Corp.) is used to measure. In the form MPC, a test liquid is spread on a paper surface and a color thereof is compared with a reference color to measure.

A thickness of the second layer is preferably from 3 to 50 µm and more preferably from 4 to 40 µm. When the thickness of the second layer is within the range, the image blurring and color mixing between colors are preferably inhibited from occurring.

### (Other Layer)

In the recording medium of the invention, other layers other than the first and second layers may be disposed as the other layer. The other layer may be appropriately selected according to the object.

### <Producing Method of Recording Medium>

The recording medium of the invention, as far as it is produced so as to have a layer structure where a first layer and a second layer are laminated sequentially from a base paper side on the base paper, is not particularly restricted in the producing method. However, the recording medium of the invention is preferably produced according to a method (producing method of a recording medium of the invention) that includes a first forming step where, on a base paper, a film-forming solution containing thermoplastic resin particles is provided, followed by heating in a temperature region equal to or more than the minimum film-forming temperature of the thermoplastic resin particles to form a first layer; and a second forming step where, on the first layer, a film-forming solution containing kaolin and polyvinyl alcohol, is provided to form a second layer. The producing method of the recording medium of the invention may further include, as needs arise, appropriately selected other steps.

### -First Forming Step-

In the first forming step, on a base paper, a film-forming solution (film-forming solution for forming a first layer) containing thermoplastic resin particles is provided, followed by heating in a temperature region equal to or more than the minimum film-forming temperature of the thermoplastic resin particles to form a first layer. In the heating step, pressure may be applied.

Details of the base paper are same as that mentioned in the first layer above and a preferable aspect as well is same.

Examples of the thermoplastic resins and particles thereof include ones same as the thermoplastic resins capable of using in the first layer and latexes thereof without particular restriction. The thermoplastic resin particles may be used singularly or in a combination of two or more kinds thereof.

It is preferable for the thermoplastic resin particle to have an average particle diameter of 10 to 200 nm. Here, the average particle diameter of thermoplastic resin particle is a value measured by a laser diffraction/dynamic light scattering method (Device name: ELS-800, manufactured by Otsuka Electronics Co., Ltd.).

Furthermore, a thermoplastic resin that constitutes the thermoplastic resin particles preferably has the minimum film-forming temperature (MFT) in the range of 5 to 60°C.

A coating amount of the thermoplastic resin is preferably in the range of 1 to 30 g/m².

The thermoplastic resin particle preferably contains, from the viewpoint of suppression of cockling, an improvement in the temporal blurring and production aptitude, dispersion particles of water dispersive latex. The water dispersive latex is one where a hydrophilic polymer insoluble or difficult to dissolve in water is dispersed as fine particles in an aqueous phase. As the dispersion state, any one of one where a polymer is emulsified in a dispersion medium, one obtained by emulsion polymerization, one obtained by micelle dispersion or one where a polymer molecule partially has a hydrophilic structure and a molecular chain per se is dispersed molecule-like may be used. The water dispersive latexes are detailed in "Gosei Jushi Emulsion (Synthetic Resin Emulsion)", edited by Taira Okuda and Hiroshi Inagaki, published by Kobunshi Kankokai (1978); "Gosei Latex no Oyo (Application of Synthetic Latexes)", edited by Takaaki Sugimura, Yasuo Kataoka, Soichi Suzuki and Keiji Kasahara, published by Kobunshi Kankokai (1993); and "Gosei Latex no Kagaku (Chemistry of Synthetic Latexes)", written by Soichi Muroi, published by Kobunshi Kankokai (1970).

Preferable specific examples of the water dispersive latex include at least one member selected from polyester urethane latex, acrylic latex, acrylic silicone latex, acrylic epoxy latex, acrylic styrene latex, acrylic urethane latex, styrene-butadiene latex, acrylonitrile-butadiene latex, and vinyl acetate latex.

A molecular weight of the water dispersive latex, by number average molecular weight, is preferably from 3,000 to 1,000,000 and particularly preferably substantially from 5,000 to 100,000. The molecular weight, when it is 3,000 or more, allows securing the mechanical strength of the first layer and, when it is 1,000,000 or less, is advantageous from the production aptitudes such as dispersion stability and viscosity.

Among the water dispersive latex, in the first layer, one member or two or more members selected from polyester urethane latex and acrylic silicone latex are the most preferable from the viewpoint that the effects of suppressing ink solvent permeability and cockling are high and both economical efficiency and production suitability are given.

A disposing method of the film-forming solution for the first layer, as far as it is capable of forming a film, is applied without particular restriction. Examples thereof include arbitrary known methods such as a coating method, an inkjet method or a dipping method. From the viewpoint of the smoothness of a film surface after film formation, a coating method that uses a film-forming solution for the first layer as a coating solution is preferred.

As the coating method, a known coating method may be applied. Examples of the known coating methods include a blade coating methods, a slide bead method, a curtain method, an extrusion method, an air knife method, a roll coating method and a rod bar coating method.

After coating, a coated film is heated in a temperature region equal to or more than the minimum film-forming temperature of the thermoplastic resin. The heating step may combine a drying step after coating or may be applied separately. The heating step is carried out according to a method were a work is put in an oven set at a temperature of the minimum film-forming temperature or more or a method where a drying air having a temperature equal to or more than the minimum film-forming temperature is blown.

### -Second Forming Step-

In the second forming step, on the first layer formed in the first forming step, a film-forming solution containing kaolin and polyvinyl alcohol (a film-forming solution for the second layer), is provided to form a second layer. Except that a second layer is formed on the first layer, there is no particular restriction; accordingly, appropriate selection may be applied depending on the object.

A disposing method of the film-forming solution for the second layer, as far as it is capable of forming a film, is applied without particular restriction. Examples thereof include arbitrary known methods such as a coating method, an inkjet method or a dipping method. From the viewpoint of capable of obtaining a smooth and highly glossy film surface after film formation, a coating method that uses a film-forming solution for the second layer as a coating solution is preferred.

As the coating method, a known coating method may be applied. Examples of the known coating methods include a blade coating method (bent method, bevel method), a slide bead method, a curtain method, an extrusion method, an air knife method, a roll coating method and a rod bar coating method. Among these, from the viewpoint of being capable of coating at a highspeed and of being capable of obtaining the glossiness by accelerating an orientation when a flat plate pigment such as a layered inorganic compound is used, a blade coating method is preferred. Furthermore, in the blade coating method, at the moment of scraping, relatively large shearing stress is generated; accordingly, due to pressure permeation due to instantaneous nip pressure, a large amount of water tends to move into a paper support. However, the blade coating method is particularly effective in the recording medium of the invention, which is provided with the first layer that blocks a solvent from permeating.

Other than the above-mentioned step, without particular restriction, other step may be disposed. The other step may be appropriately selected depending on the object.

### <Inkjet Recording Method>

An inkjet recording method of the invention may be constituted by disposing an ink drawing step where ink is provided to the recording medium of the invention to apply ink drawing in accordance with predetermined image data and a drying and removing step where an ink solvent in the ink drawn recording medium is dried and removed.

For example, an inkjet recording method (see Fig. 2; hereinafter, referred to as an "inkjet recording method involving the first aspect") that applies the ink drawing to, among the recording media of the invention, a recording medium in which a coagulant (treatment solution) is previously added in the second layer (coated layer on the first layer) to lower the pH of a layer surface, and an inkjet recording method (see Fig. 3; hereinafter, referred to as a "inkjet recording method involving the second aspect") where, after a treatment solution containing an acidic substance is fed (pre-coat) to the recording medium of the invention, the ink drawing is applied are cited.

An inkjet recording method involving the first exemplary embodiment of the invention is constituted by including an ink drawing step where ink is provided to a recording medium of the invention where the pH of a layer surface of the second layer is controlled to 4 or less to apply ink drawing in accordance with predetermined image data and a drying and removing step where an ink solvent in the ink drawn recording medium is dried to remove.

Furthermore, an inkjet recording method involving the second aspect of the invention is constituted by including a treatment solution feed step where a treatment solution containing an acidic substance is fed to the recording medium of the invention, an ink drawing step where ink is provided to the recording medium to which the treatment solution is fed to apply ink drawing in accordance with predetermined image data and a drying and removing step where an ink solvent in the ink drawn recording medium is dried to remove.

All of the inkjet recording methods involving the first and second aspects may, as needs arise, contain appropriately selected other step.

### -Ink Drawing Step-

In the ink drawing step of the first aspect, among the recording media mentioned above, a recording medium of the invention where a layer surface of the second layer is controlled to the pH of 4 or less is used, and ink is provided to the second layer of the recording medium to apply ink drawing in accordance with predetermined image data. When the ink (such as pigment ink) is provided to the second layer, the ink (such as pigment in ink) is coagulated owing to the pH variation at the time of ink striking to inhibit the ink from causing the blurring and color mixing between colors.

In the ink drawing step of the second aspect, without controlling the pH of a layer surface of the second layer to 4 or less or with the pH controlling like the first aspect, ink is provided to a recording medium to which a treatment solution is fed in the treatment solution feed step described below to apply the ink drawing in accordance with predetermined image data. In the second aspect, before the ink is provided or at the same time with the ink provision, the second layer is at least partially rendered acidic (preferably pH is 4 or less) due to the treatment solution fed to the second layer; accordingly, the ink (such as pigment ink) provided thereto undergoes a pH variation at the time of droplet impact to coagulate to inhibit the ink from causing the blurring and color mixing between colors.

The ink drawing step has no particular restriction other than drawing is carried out by providing ink in accordance with the predetermined image data and may be appropriately selected in accordance with the object. For instance, ink is discharged by use of an inkjet method to apply the ink drawing. The inkjet recording method is not particularly restricted and any one of an electric charge control method where ink is discharged by making use of force of electrostatic attraction, a drop-on demand method (pressure pulse method) that makes use of vibration pressure of a piezo device, an acoustic inkjet method where an electric signal is converted into an acoustic beam to illuminate ink and by making use of radiation pressure ink is discharged and a thermal inkjet method where ink is heated to generate foams to make use of generated pressure may be used. The inkjet recording method includes a method where ink called a photo-ink and low in a concentration is discharged a lot in small volume, a method where a plurality of inks substantially same in hue and different in the concentration is used to improve image quality and a method where colorless transparent ink is used.

Among the methods, a drop-on demand method (pressure pulse method) that uses a piezo device is preferred.

### -Treatment Solution Feed Step-

In the inkjet recording method involving the second aspect, before the ink drawing step, a treatment solution feed step is disposed to feed a treatment solution containing an acidic substance in advance to the second layer of the recording medium. The treatment solution feed step is not particularly restricted other than feeding a treatment solution containing the acid substance described below and may be appropriately selected depending on the object. Furthermore, the treatment solution feed step may be provided, as needs arise, to the inkjet recording method involving the first aspect.

### (Treatment Solution)

A treatment solution containing an acidic substance may well be a liquid controlled so as to have a liquid property on an acidic side by containing an acidic substance and an aqueous treatment solution obtained by mixing an acidic substance and an aqueous solvent is preferred. The pH of the treatment solution in the invention is, from the viewpoint of inhibiting the ink from causing blurring and color mixing between colors, preferably 4 or less.

Examples of the acidic substances that render the treatment solution acidic include compounds having a group such as a phosphoric acid group, a phosphonic acid group, a phosphinic acid group, a sulfuric acid group, a sulfonic acid group, a sulfinic acid group and a carboxylic acid group or a group derived from the salt thereof, a compound having a phosphoric avid group or a carboxylic acid group being preferred and a compound having a carboxylic acid group being more preferred.

Examples of compounds that have a phosphoric acid group include phosphoric acid, polyphosphoric acid or derivatives of compounds thereof, or salts thereof. Examples of compounds that have a carboxylic acid group include compounds that have a furan, pyrrole, pyrroline, pyrolidone, pyrone, pyrrole, thiophene, indole, pyridine or quinoline structure and has a carboxyl group as a functional group such as pyrolidone carboxylic acid, pyrone carboxylic acid, pyrrole carboxylic acid, furan carboxylic acid, pyridine carboxylic acid, coumaric acid, thiophene carboxylic acid, nicotinic acid, or derivatives of compounds thereof, or salts thereof. One of these is added to the treatment solution.

Furthermore, preferable examples of the acidic substances include pyrolidone carboxylic acid, pyrone carboxylic acid, furan carboxylic acid, coumaric acid or a compound derivative thereof or a salt thereof. The acidic substances may be used singularly or in a combination of two or more kinds thereof.

The treatment solution may contain, within a range that does not damage advantages of the invention, other additives.

Examples of the other additives include known additives such as a drying inhibitor (wetting agent), a discoloring inhibitor, an emulsion stabilizer, a permeation accelerator, a UV absorber, an antiseptic, a mold inhibitor, a pH adjusting agent, a surface tension adjusting agent, a defoaming agent, a viscosity adjuster, a dispersing agent, a dispersion stabilizer, a rust inhibitor or a chelating agent.

The treatment solution may be fed over an entirety of a recording surface of the Recording medium or at least partially on a recording surface such as in accordance with predetermined image data. Furthermore, a method of feeding the treatment solution is not particularly restricted. A coating method, an inkjet method and a dipping method are cited. For instance, the inkjet method may be used to discharge the treatment solution to feed.

Furthermore, in the inkjet recording method involving the second aspect, aqueous two liquid coagulating ink described below may be used to draw.

### -Drying and Removing Step-

In the drying and removing step, an ink solvent in the ink drawn recording medium is dried to remove. There is no particular restriction except that an ink solvent of the ink provided to the recording medium is dried to remove; accordingly, an appropriate selection may be applied depending on the object.

The drying and removing step is applied, since a coated layer as the second layer is mildly permeative in the recording medium of the invention, in a state where an ink solvent (water in particular) is present in the proximity of a surface of the recording medium. The drying and removing step may be applied according to a method where a dry air heated at a predetermined temperature is blown or a method where the recording medium is passed through between a pair of heated and/or pressurized rolls.

### -Other Step-

The inkjet recording method of the invention may be provided with, in addition to the above-mentioned steps, other steps. The other step is not particularly restricted and may be appropriately selected depending on the object. For instance, a heating and fixing step is cited.

In the inkjet recording method of the invention, after the drying and removing step, for instance, a heating and fixing step for melting and fixing latex particles contained in the ink used in the inkjet recording method may be disposed. According to the heating and fixing step, the fixability of the ink to the recording medium may be enhanced. The heating and fixing step is not particularly restricted except for the melting and fixing as mentioned above and may be appropriately selected depending on the object.

### -Example of Aspect of First Inkjet Recording Method-

In the first inkjet recording method, for instance, under the conditions described below, ink drawing, drying (water drying, air blow drying) and heating and fixing are carried out.

### <Ink Drawing>

Head: 1,200 dots per 2.54 cm/0.51 m (1,200 dpi/20 inch) width full-line head
Amount of discharge liquid droplet: four value recording of 0, 2.0, 3.5 and 4.0 pL
Drive frequency: 30 kHz (conveying speed of recording medium: 635 mm/sec)

### <Drying (water drying, air blow drying)>

Speed of wind: 8 to 15 m/s
Temperature: 40 to 80°C
Air blow region: 640 mm (drying time: 1 sec)

### <Heating and Fixings>

Silicone rubber roller (hardness: 50°, nip width: 5 mm)
Roller temperature: 70 to 90°C
Pressure: 0.5 to 2.0 MPa

### -Example of Aspect of Second inkjet Recording Method-

In the second inkjet recording method, for instance, under the conditions described below, pre-coating, ink drawing, drying (water drying, air blow drying) and heating and fixing are carried out.

### <Head for Treating Solution for Pre-coat Module>

Head: 600 dots per 2.54 cm/0.51 cm (600 dpi/20 inch) width full-line head
Amount of discharge liquid droplet: two value recording of 0 and 4.0 pL
Drive frequency: 15 kHz (conveying speed of recording medium: 635 mm/sec)
Drawing pattern: in the ink drawing Step, a pattern by which at a position where color ink having at least one color is drawn, a treatment solution is provided in advance is applied

### <Water-drying (air blow drying) for Pre-coat Module>

Speed of wind: 8 to 15 m/s
Temperature: 40 to 80°C
Air blow region: 450 mm (drying time: 0.7 sec)

### <Ink Drawing>

Head: 1,200 dots per 2.54 cm/0.51 cm 1,200 dpi/20 inch width full-line head
Amount of discharge liquid droplet: four value recording of 0, 2.0, 3.5 and 4.0 pL
Drive frequency: 30 kHz (conveying speed of recording medium: 635 mm/sec)

### <Drying (water drying, air blow drying)>

Speed of wind: 8 to 15 m/s
Temperature: 40 to 80°C
Air blow region: 640 mm (drying time: 1 sec)

### <Heating and Fixing>

Silicone rubber roller (hardness: 50°, nip width: 5 mm)
Roller temperature: 70 to 90°C
Pressure: 0.5 to 2.0 MPa

### ~aqueous Two-liquid Coagulating Ink~

In the inkjet recording method involving the second aspect, aqueous two liquid coagulating ink including a treatment solution and ink that reacts with the treatment solution to coagulate may be used.

As the treatment solution of the aqueous two liquid coagulating ink, one similar to the above-mentioned treatment solution may be used. Details of the treatment solution are as mentioned above.

### -Ink-

The ink which constitutes aqueous two-liquid coagulating ink system can be used in not only monochromatic image formation, but full color image formation. To form a full color image, a magenta tone ink, a cyan tone ink and a yellow tone ink can be used, and to adjust the tone, a black tone ink may further be used. Furthermore, other than the yellow, magenta and cyan tone inks, red, green, blue and white color inks and so-called specific color inks in printing filed (for example, colorless) can be used.

Furthermore, as the ink, one that contains, for instance, latex particles, an organic dye, a dispersing agent and an aqueous organic solvent, and, as needs arise, further contains other additives is cited.

### <Latex Particles>

As the latex particles, particles of a polymer of a compound made of, for instance, a nonionic monomer, an anionic monomer or a cationic monomer, which is dispersed in an aqueous medium, are cited.

The nonionic monomer means a monomer compound that does not have a dissociative functional group. The monomer compound means in the broad sense a polymerizable compound alone or a compound that polymerizes with another compound. As the monomer compound, a monomer compound having an unsaturated double bond is cited.

The anionic monomer means a monomer compound that contains an anionic group capable of having a minus charge. The anionic group, as far as it has a minus charge, may be any one, and preferable examples thereof include a phosphoric acid group, a phosphonic acid group, a phosphinic acid group, a sulfuric acid group, a sulfonic acid group, a sulfinic acid group and a carboxylic acid group, a phosphoric acid group and a carboxylic acid group being more preferred, and a carboxylic acid group being further more preferred.

The cationic monomer means a monomer containing a cationic group capable of having a plus charge. The cationic group, as far as it has a plus charge, may be any one. However, an organic cationic substituent is preferred and a cationic group of nitrogen or phosphorus is more preferred. Furthermore, a pyridinium cation or ammonium cation is more preferred.

### <Organic pigments>

Examples of the organic pigment for orange or yellow include C.I. Pigment Orange 31, C.I. Pigment Orange 43, C.I. Pigment Yellow 12, C.I. Pigment Yellow 13, C.I. Pigment Yellow 14, C.I. Pigment Yellow 15, C.I. Pigment Yellow 17, C.I. Pigment Yellow 74, C.I. Pigment Yellow 93, C.I. Pigment Yellow 94, C.I. Pigment Yellow 128, C.I. Pigment Yellow 138, C.I. Pigment Yellow 151, C.I. Pigment Yellow 155, C.I. Pigment Yellow 180 and C.I. Pigment Yellow 185.

Examples of the organic pigment for magenta or red include C.I. Pigment Red 2, C.I. Pigment Red 3, C.I. Pigment Red 5, C.I. Pigment Red 6, C.I. Pigment Red 7, C.I. Pigment Red 15, C.I. Pigment Red 16, C.I. Pigment Red 48:1, C.I. Pigment Red 53:1, C.I. Pigment Red 57:1, C.I. Pigment Red 122, C.I. Pigment Red 123, C.I. Pigment Red 139, C.I. Pigment Red 144, C.I. Pigment Red 149, C.I. Pigment Red 166, C.I. Pigment Red 177, C.I. Pigment Red 178, C.I. Pigment Red 222 and C.I. Pigment Violet 19.

Examples of the organic pigment for green or cyan include C.I. Pigment Blue 15, C.I. Pigment Blue 15:2, C.I. Pigment Blue 15:3, C.I. Pigment Blue 15:4, C.I. Pigment Blue 16, C.I. Pigment Blue 60, C.I. Pigment Green 7, and siloxane-crosslinked aluminum phthalocyanine described in US Patent 4,311,775.

Examples of the organic pigment for black include C.I. Pigment Black 1, C.I. Pigment Black 6 and C.I. Pigment Black 7.

Furthermore, an average particle diameter of an organic pigment is preferred to be smaller from the viewpoint of the transparency and color reproducibility and preferred to be larger from the viewpoint of the light resistance. An average particle diameter that combines these requirements is preferably from 10 to 200 nm, more preferably from 10 to 150 nm and still more preferably from 10 to 100 nm. Still furthermore, a particle size distribution of the organic pigment is not restricted to particular one. Any one of one that has a broad particle size distribution and one that has a mono-disperse particle size distribution may be used. Furthermore, two or more kinds of organic pigments having a mono-disperse particle distribution may be mixed and used.

Furthermore, an addition amount of the organic pigment is, relative to the ink, preferably from 1 to 25% by mass, more preferably from 2 to 20% by mass, still more preferably from 5 to 20% by mass and particularly preferably from 5 to 15% by mass.

### <Dispersant>

The dispersant for the organic pigment may be a polymer dispersant, or a low molecular surfactant type dispersant. The polymer dispersant may be either one of a water-soluble dispersant or a water-insoluble dispersant.

The low molecular surfactant type dispersant can be added for the purpose of stably dispersing the organic pigment in a water solvent while maintaining an ink in low viscosity. The low molecular dispersant used herein means a low molecular dispersant having A molecular weigh of 2,000 or lower. The molecular weight of the low molecular weight dispersant is preferably from 100 to 2,000, and more preferably from 200 to 2,000.

The low molecular dispersant has a structure containing a hydrophilic group and a hydrophobic group. At least one of each of the hydrophilic group and the hydrophobic group may be independently contained in one molecule, and the low molecular dispersant may have plural kinds of the hydrophilic group and the hydrophobic group. The low molecular dispersant can appropriately have a linking group for linking the hydrophilic group and the hydrophobic group.

Examples of the hydrophilic group include an anionic group, a cationic group, a nonionic group, and a betaine type combining those.

The anionic group is not particularly limited so long as it has a negative charge. A phosphoric acid group, a phosphonic acid group, a phosphinic acid group, a sulfuric acid group, a sulfonic acid group, a sulfinic acid group and a carboxyl group are preferred, a phosphoric acid group and carboxyl group are more preferred, and a carboxyl group is further preferred. The cationic group is not particularly limited so long as it has a positive charge. An organic cationic substituent is preferred, a cationic group containing nitrogen or phosphorus is more preferred. Above all, pyridinium cation and ammonium cation are particularly preferred.

Examples of the nonionic group include polyethylene oxide, polyglycerin and a part of sugar unit

It is preferred in the invention that the hydrophilic group is an anionic group from the standpoints of dispersion stability and aggregation properties of a pigment. A phosphoric acid group, a phosphonic acid group, a phosphinic acid group, a sulfuric acid group, a sulfonic acid group, a sulfinic acid group and a carboxyl group are preferred as the anionic group, a phosphoric acid group and carboxyl group are more preferred, and a carboxyl group is further preferred.

When the low molecular dispersant has an anionic hydrophilic group, its pKa is preferably 3 or more from the standpoint of accelerating an aggregation reaction by contacting with an acidic treating liquid. The pKa of the low molecular dispersant in the invention is a value experimentally obtained from a titration curve by titrating a liquid obtained dissolving 1 mmol/liter of a low molecular dispersant in a tetrahydrofuran-water=3:2 (V/V) solution, with an acid or alkali aqueous solution.

Theoretically, when pKa of a low molecular weight dispersant is 3 or more, 50% or more of anionic groups are in a non-dissociation state when contacted with a treating liquid having a pH of about 3. Therefore, water solubility of the low molecular weight dispersant is remarkably decreased, and an aggregation reaction occurs. In other words, aggregation reactivity is improved. From this standpoint, it is preferred that the low molecular dispersant has a carboxylic group as an anionic group.

The hydrophobic group may have any structure of hydrocarbon type, fluorocarbon type, silicone type and the like, and the hydrocarbon type is particularly preferred. Those hydrophobic groups may have any of a linear structure and a branched structure. The hydrophobic group may have one chain structure or two or more chain structure. Where the structure has two or more chains, the structure may have plural kinds of hydrophobic groups. The hydrophobic group is preferably a hydrocarbon group having 2 to 24 carbon atoms, more preferably a hydrocarbon group having 4 to 24 carbon atoms, further preferably a hydrocarbon group having 6 to 20 carbon atoms.

Among the polymer dispersants, a hydrophilic polymer compound can be used as the water-soluble dispersant. Examples of a natural hydrophilic polymer compound include vegetable polymers such as gum Arabic, gum tragacanth, gum guar, gum karaya, locust bean gum, arabinogalactan, pectin and quince seed starch; seaweed polymers such as alginic acid, carrageenan and agar; animal polymers such as gelatin, casein, albumin and collagen; and microbial polymers such as xanthene gum and dextran.

Examples of a modified hydrophilic polymer compound using a natural product as a raw material include cellulose polymers such as methyl cellulose, ethyl cellulose, hydroxyethyl cellulose, hydroxypropyl cellulose and carboxymethyl cellulose; starch polymers such as starch sodium glycolate and starch sodium phosphate ester; and seaweed polymers such as sodium alginate, propylene glycol alginate ester.

Examples of a synthetic water-soluble polymer compound include vinyl polymers such as polyvinyl alcohol, polyvinyl pyrrolidone and polyvinyl methyl ether; acrylic resins such as non-crosslinked polyacrylamide, polyacrylic acid or its alkali metal salt, and water-soluble styrene acrylic resin; water-soluble styrene maleic acid resins; water-soluble vinylnaphthalene acrylic resins; water-soluble vinylnaphthalene maleic resins; polyvinyl pyrrolidone, polyvinyl alcohol, alkali metal salts of β-naphthalenesulfonic acid formalin condensate; polymer compounds having a salt of a cationic functional group such as quaternary ammonium or amino group at a side chain; and natural polymers such as shellac.

Among these, one obtained by introducing a carboxyl group like one made of a homopolymer of acrylic acid or methacrylic acid or a copolymer of acrylic acid or methacrylic acid with styrene or a monomer that has other hydrophilic group is particularly preferred as a polymer dispersing agent.

Of the polymer dispersants, as a non-water-soluble dispersant, a polymer having both a hydrophilic moiety and a hydrophobic moiety may be used. Examples of such a polymer include styrene-(meth)acrylic acid copolymer, styrene-(meth)acrylic acid-(meth)acrylic acid ester copolymer, (meth)acrylic acid ester-(meth)acrylic acid copolymer, polyethylene glycol (meth)acrylate-(meth)acrylic acid copolymer, vinyl acetate-maleic acid copolymer and styrene-maleic acid copolymer.

The polymer dispersant used in the invention has a weight average molecular weight of preferably from 3,000 to 100,000, more preferably from 5,000 to 50,000, further preferably from 5,000 to 40,000, and particularly preferably from 10,000 to 40,000.

Mixing mass ratio of an organic pigment and a dispersant (pigment:dispersant) is preferably in a range of from 1:0.06 to 1:3, more preferably in a range of from 1:0.125 to 1:2, and further preferably in a range of from 1:0.125 to 1:1.5.

### (Water-soluble organic solvent)

The water-soluble organic solvent can be contained as a drying inhibitor or a permeation accelerator.

Where the water-based ink composition of the invention is particularly applied to an image recording method by an inkjet method, the drying inhibitor can effectively prevent clogging of nozzle that may possibly be generated by drying of an ink at an ink jet orifice.

The drying inhibitor is preferably a water-soluble organic solvent having vapor pressure lower than that of water. Specific examples of the drying inhibitor include polyhydric alcohols such as ethylene glycol, propylene glycol, diethylene glycol, polyethylene glycol, thiodiglycol, dithiodiglycol, 2-methyl-1,3-propanediol, 1,2,6-hexanetriol, acetylene glycol derivatives, glycerin and trimethylolpropane; lower alkyl ethers of polyhydric alcohol, such as ethylene glycol monomethyl (or ethyl) ether, diethylene glycol monomethyl (or ethyl) ether and triethylene glycol monoethyl (or butyl) ether; heterocycles such as 2-pyrrolidone, N-methyl-2-pyrrolidone, 1,3-dimethyl-2-imidazolidinone and N-ethylmorpholine; sulfur-containing compounds such as sulfolane, dimethylsufoxide and 3-sulforene; polyfunctional compounds such as diacetone alcohol and diethanolamine; and urea derivatives. Above all, polyhydric alcohols such as glycerin and diethylene glycol are preferred as the drying inhibitor. Those drying inhibitors may be used alone or as mixtures of two kinds or more thereof. Those drying inhibitors are preferably contained in an amount of from 10 to 50% by mass in the ink.

The water-soluble organic solvent as the permeation accelerator is preferably used for the purpose of well permeating the ink into a recording medium (printing paper). Specific examples of the permeation accelerator include alcohols such as ethanol, isopropanol, butanol, di(tri)ethylene glycol monobutyl ether and 1,2-hexanediol; sodium lauryl sulafate, sodium oleate and nonionic surfactants. When the permeation accelerator is contained in the ink composition in an amount of from 5 to 30% by mass, sufficient effect is exhibited. The permeation accelerator is preferably used within a range of the addition amount such that bleeding of printing and print-through are not generated.

The water-soluble organic solvent can be used to adjust viscosity, other than the above. Specific examples of the water-soluble organic solvent that can be used to adjust viscosity include alcohols (for example, methanol, ethanol, propanol, isopropanol, butanol, isobutanol, sec-butanol, t-butanol, pentanol, hexanol, cyclohexanol and benzyl alcohol), polyhydric alcohols (for example, ethylene glycol, diethylene glycol, triethylene glycol, polyethylene glycol, propylene glycol, dipropylene glycol, polypropylene glycol, butylene glycol, hexanediol, pentanediol, glycerin, hexanetriol and thiodiglycol), glycol derivatives (for example, ethylene glycol monomethyl ether, ethylene glycol monoethyl ether, ethylene glycol monobutyl ether, diethylene glycol monomethyl ether, diethylene glycol monobutyl ether, propylene glycol monomethyl ether, propylene glycol monobutyl ether, dipropylene glycol monomethyl ether, triethylene glycol monomethyl ether, ethylene glycol diacetate, ethylene glycol monomethyl ether acetate, triethylene glycol monomethyl ether, triethylene glycol monoethyl ether and ethylene glycol monophenyl ether), amines (for example, ethanolamine, diethanolamine, triethanolamine, N-methyl diethanolamine, N-ethyl diethanolamine, morpholine, N-ethylmorpholine, ethylene diamine, diethylene triamine, triethylene tetramine, polyethylene imine and tetramethylpropylene diamine), and other polar solvents (for example, formaldehyde, N,N-dimethylformamide, N,N-dimethylacetamide, diemthylsulfoxide, sulfolane, 2-pyrrolidone, N-methyl-2-pyrrolidone, N-vinyl-2-pyrrolidone, 2-oxazolidone, 1,3-dimethyl-2-imidazolidinone, acetonitrile and acetone).

The water-soluble organic solvent may be used alone or as mixtures of two kinds or more thereof.

### (Other additives)

Examples of other additives used in the invention include conventional additives such as drying inhibitor (wetting agent), color fading inhibitor, emulsion stabilizer, permeation accelerator, ultraviolet absorber, preservative, mildew-proofing agent, pH regulator, surface tension regulator, defoamer, viscosity regulator, dispersant, dispersion stabilizer, anti-rust agent and chelating agent.

The various kinds of the additives, in the case of an aqueous ink, are added directly to the ink. In the case where an oil-soluble dye is used in the form of a dispersion, it is general that, after a dye dispersion is prepared, the additive is added to the dispersion. However, during preparation of the dye dispersion, the additive may be added to an oil phase or an aqueous phase.

The ultraviolet absorber is used for the purpose of improving preservability of an image. The ultraviolet absorber can use benzotriazole compounds described in, for example, JP-A Nos. 58-185677, 61-190537, 2-782, 5-197075 and 9-34057; benzophenone compounds described in, for example, JP-A Nos. 46-2784 and 5-194483, and US Patent No. 3,214,463; cinnamic acid compounds described in, for example, JP-B Nos. 48-30492 and 56-21141, and JP-A No. 10-88106; triazine compounds described in, for example, JP-A Nos. 4-298503, 8-53427, 8-239368 and 10-182621, and JP-A No. 8-501291; compounds described in Research Disclosure No. 24239; and compounds that absorb ultraviolet light and emit fluorescence, i.e., fluorescent brighteners, represented by stilbene compounds or benzoxazole compounds.

The color fading inhibitor is used for the purpose of improving storability of an image. Examples of the color fading inhibitor that can be used include various organic color fading inhibitors and metal complex color fading inhibitors. Examples of the organic color fading inhibitor include hydroquinones, alkoxyphenols, dialkoxyphenols, phenols, anilines, amines, indanes, chromanes, alkoxyanilines and heterocycles. Examples of the metal complex color fading inhibitor include a nickel complex and a zinc complex. More specifically, compounds described in the patents cited in Research Disclosure No. 17643, chapter VII, items I to J; Research Disclosure No. 15162: Research Disclosure No. 18716, page 650, the left-hand column; Research Disclosure No. 36544, page 527; Research Disclosure No. 307105, page 872; and Research Disclosure No. 15162, and compounds included in the formulae of the representative compounds and the exemplified compounds described on pages 127 to 137 of JP-A No. 62-215272 can be used.

Examples of the mildew-proofing agent include sodium dehydroacetate, sodium benzoate, sodium pyridinethion-1-oxide, p-hydroxybenzoic acid ethyl ester, 1 ,2-benzisothiazolin-3-one and its salt. Those are preferably used in the ink composition in an amount of from 0.02 to 1.00% by mass.

As the pH regulator, a neutralizer (organic base and inorganic alkali) may be used. The pH regulator may be added in an amount such that the inkjet ink composition has pH of preferably from 6 to 10, and more preferably from 7 to 10, for the purpose of improving storage stability of the inkjet ink composition.

Examples of the surface tension regulator include nonionic surfactants, cationic surfactants, anionic surfactants and betaine surfactants.

The surface tension regulator is added in an amount such that the surface tension of the ink composition is adjusted to preferably from 20 to 60 mN/m, more preferably from 20 to 45 mN/m, and further preferably from 25 to 40 mN/m, in order to well eject the ink composition by an inkjet method.

Specific examples of the surfactant as a hydrocarbon type preferably include anionic surfactants such as fatty acid salts, alkyl sulfate ester salts, alkyl benzene sulfonates, alkyl naphthalene sulfonates, dialkyl sulfosuccinates, alkyl phosphate ester salts, naphthalenesulfonic acid-formalin condensates and polyoxyethylene alkyl sulfate ester salts; and nonionic surfactants such as polyoxyethylene alkyl ether, polyoxyethylene alkyl allyl ether, polyoxyethylene fatty acid ester, sorbitan fatty acid ester, polyoxyethylene sorbitan fatty acid ester, polyoxyethylene alkyl amine, glycerin fatty acid ester and oxyethylene oxypropylene block copolymer. SURFYNOLS (trade name, products of Air Products & Chemicals) which are an acetylene type polyoxyethylene oxide surfactant are preferably used. Furthermore, amine oxide type amphoteric surfactants such as N,N-dimethyl-N-alkyl amine oxide are preferred.

Additionally, materials described on pages (37) to (38) of JP-A No. 59-157636 and Research Disclosure No. 308119 (1989) as surfactants can be used.

When fluorine (alkyl fluoride type) surfactants, silicone surfactants and the like, such as those described in JP-A Nos. 2003-322926, 2004-325707 and 2004-309806 are used, scratch fastness can be improved.

The surface tension regulator can be used as a defoamer, and fluorine compounds, silicone compounds, chelating agents represented by EDTA, and the like can be used.

### EXAMPLES

In what follows, the present invention will be more specifically described with reference to examples. However, the invention is defined by the claims and is not restricted to examples shown below. Herein, unless stated clearly, "part" and "%" are based on mass and "degree of polymerization" expresses an "average degree of polymerization".

### [Example 1]

### <Preparation of Inkjet Recording Medium>

### (Preparation of Film-forming Solution for First Layer)

In the beginning, 100 parts of kaolin (trade name: KAOBRIGHT 90, manufactured by SHIRAISHI CALCIUM KAISHA, LTD.), 3.8 parts of 0.1 N sodium hydroxide (Wako Pure Chemical Industries, Limited), 1.2 parts of 40% sodium polyacrylate (trade name: ARON T-50, manufactured by TOAGOSEI CO., LTD.) and 48.8 parts of water were mixed and dispersed by use of a non-bubbling kneader (trade name: NBK-2, manufactured by Nippon Seiki Co., Ltd.), thereby, a 65% kaolin dispersion was obtained. In the next place, to 100 parts of 22.5% polyester urethane latex aqueous dispersion (glass transition temperature: 49°C, the minimum film-forming temperature: 29°C; trade name: HYDRAN AP-40F, manufactured by DIC Corporation), 5 parts of water, 6.9 parts of the resulting 65% kaolin dispersion and 0.8 parts of 10% Emulgen 109P (trade name, manufactured by KAO CORPORATION) were added, followed by thoroughly agitating and mixing, further followed by maintaining a resulting mixed solution at a liquid temperature from 15 to 25°C, thereby a 24.0% coating liquid for forming a first layer was obtained.

### (Preparation of a coating liquid for a second layer)

100 parts of kaolin (Tradename: Kaobright 90, produced by Shiraishi Calcium Kaisha, Ltd.) and 1.2 parts of 40% sodium polyacrylate (Tradename: Aaron T-50, manufactured by Toagosei Chemical Industry Co.) were mixed and dispersed in water. Then, to the resultant, 100 parts of 7% aqueous PVA245 solution (manufactured by Kuraray) and 3.7 parts of 10% aqueous emulgen 109P solution (manufactured by Kao Corporation) were added to prepare a coating liquid having a final solid content of 27% for a second layer.

### (Formation of a first layer)

To both sides of fine paper (Tradename: "Shiraoi", manufactured by Nippon Paper Industries) having a basis weight of 81.4 g/m², the obtained coating liquid for a first layer was applied to one side and then another side using an extrusion die coater while adjusting the coating amount per one side to 8.0 g/m². Then the resultant was dried for 1 minute at a temperature of 85°C and at a wind velocity of 15 m/sec to form a first layer. Furthermore, the formed first layer was subjected to soft calender treatment described below. The thickness of the formed first layer was 8.1 µm.

### -Soft Calender Treatment-

To a high-quality paper on a surface of which a first layer was formed, by use of a soft calender provided with a roll pair where a metal roll and a resin roll are paired, under conditions of a surface temperature of the metal roll of 50°C and nip pressure of 50 kg/cm, a soft calender process was applied.

### (Formation of Second Layer)

On both sides of a high-quality paper on which the first layer was formed, an obtained film-forming solution for the second layer was coated on one surface at a time by use of an extrusion die-coater with a dry mass per one surface controlling so as to be 30 g/m², followed by drying at a temperature of 70°C and a speed of wind of 10 m/sec for 1 min, thereby, a second layer was formed. Similarly to the case of the first layer, a soft calender treatment was applied to the formed second layer. A thickness of the formed second layer was 20.2 µm.

Thus, an inkjet recording medium of the invention was prepared.

### (Evaluation)

Resulting inkjet recording medium was subjected to evaluations 1. through 5. below. Evaluation results are shown in Table 1 below.

### -1. Cobb's Water Absorbency Test-

According to the Cobb's water absorbency test based on JIS P8140, at a surface of a first layer of a high-quality paper on which a first layer was formed, the Cobb's water absorbency (a permeating amount of water when water was brought into contact at 20°C for 2 minutes (g/m²)) was measured.

### -2. Water Absorbency Test for the Second Layer-

Based on the Bristow method, a measurement was carried out as shown below.

A sample piece of the second layer obtained by cutting an obtained inkjet recording medium into A6 size was set on a measurement table. After a head filled with a test solution was brought into contact with a disposed sample piece, a scanning line (from inside to outside) as shown in Fig. 4 was automatically scanned to measure the liquid absorption characteristics. By rotating a measurement table with a revolution speed (contact time of paper and ink) varying stepwise, relationship between the contact time and amount of absorbed liquid (amount of absorbed water) was obtained. In Table 1 below, amounts of absorbed water at a contact time of 0.5 sec were shown.

### -3. Curl Test-

An inkjet recording medium was cut into a size of 50 mm x 50 mm to prepare a test piece, water was coated on the test piece to the respective directions of MD and CD so as to be 10 g/m², and, based on a curl curvature measurement method stipulated in JAPAN TAPPI Paper and Pulp Test Method No. 15-2: 2000 (Paper-curl Test Method-Second Part), the curling degree when left for 8 hr under environmental conditions of 23 °C and 50% RH was evaluated according to criteria blow.

### <Evaluation Criteria>

A: The curling degree was less than 10.
B: The curling degree was 10 or more and less than 20.
C: The curling degree was 20 or more and less than 30.
D: The curling degree was 30 or more.

### <Preparation of Ink>

### (1) Preparation of Cyan Pigment Ink C

### -Preparation of Pigment Dispersion-

In the beginning, 10 g of CYANINE BLUE A-22 (PB15: 3) (trade name, manufactured by Dainichiseika Color & Chemicals Mfg. Co., Ltd.), 10.0 g of a low molecular weight dispersing agent described below, 4.0 g of glycerin and 26 g of ion exchange water were agitated and mixed to prepare a dispersion. In the next place, the dispersion was intermittently irradiated (irradiation 0.5 sec/non-irradiation 1.0 sec) with ultrasonic wave by use of an ultrasonic irradiation apparatus (VIBRA-CELL VC-750 made by Sonics Inc.., tapered microchips: φ 5 mm, amplitude: 30%) for two hours to further disperse the pigment therein, thereby a 20% by mass pigment dispersion was prepare

Low molecular weight dispersing agent

Separately from the pigment dispersion, the compounds shown below were weighed, agitated and mixed to prepare a mixture solution I.
· glycerin ... 5.0 g
· diethylene glycol ... 10.0 g
· OLFINE E1010 (trade name, manufactured by Nisshin Chemical Industry Co. Ltd.)... 1.0 g
· ion exchange water ... 11.0 g

The mixture solution I was gradually added dropwise to 23.0 g of a 44% SBR dispersion (polymer fine particles: acrylic acid 3%, Tg (glass transition temperature): 30°C) which was agitated, followed by agitating and mixing, thereby a mixture solution II was obtained.

Then, the mixture solution II was agitated and mixed while gradually adding dropwise to a 20% by mass pigment dispersion, and, thereby 100 g of cyan pigment ink C (cyan ink) was prepared. By use of a pH meter WM-50EG (trade name, manufactured by DKK-TOA CORPORATION), the pH of the pigment ink C prepared as mentioned above was measured and a pH value thereof was 8.5.

### (2) Preparation of Magenta Pigment Ink M

Except that, in the preparation of the pigment ink C, in place of a pigment used in the preparation of the pigment ink C; CROMOPHTAL JET MAGENTA DMQ (PR-122) (trade name, manufactured by Ciba Specialty Chemicals Inc.) was used, according to a method similar to that of the pigment ink C, magenta pigment ink M (magenta ink) was prepared. By use of a pH meter WM-50EG (trade name, manufactured by DKK-TOA CORPORATION), the pH of the pigment ink M prepared as mentioned above was measured and a pH value thereof was 8.5.

### (3) Preparation of Yellow Pigment Ink Y

Except that, in the preparation of a pigment ink C, in place of a pigment used in the preparation of the pigment ink C, IRGALITE YELLOW GS (PY74) (trade name, manufactured by Ciba Specialty Chemicals Inc.) was used, according to a method similar to that of the pigment ink C, yellow pigment ink Y (yellow ink) was prepared. By use of a pH meter WM-50EG (trade name, manufactured by DKK-TOA CORPORATION), the pH of the pigment ink Y prepared as mentioned above was measured and a pH value thereof was 8.5.

### (4) Preparation of Black Pigment Ink K

Except that, in the preparation of a pigment ink C, in place of a pigment dispersion used in the preparation of the pigment ink C, CAB-O-JETTM_200 (carbon black) (trade name, manufactured by Cabot Corporation.) was used, according to a method similar to that of the pigment ink C, black pigment ink K (black ink) was prepared. By use of a pH meter WM-50EG (trace name, manufactured by DKK-TOA CORPORATION), the pH of the pigment ink K prepared as mentioned above was measured and a pH value was 8.5.

### <Preparation of Treatment Solution>

A treatment solution was prepared by mixing components shown below.
phosphoric acid 10 g
glycerin 20 g
diethylene glycol 10 g
OLFINE E1010 (manufactured by Nisshin Chemical Industry Co. Ltd.) 1 g
ion exchange water 59 g

By use of a pH meter WM-60EG (trade name, manufactured by DKK-TOA CORPORATION), the pH of the treatment solution prepared as mentioned above was measured and a pH value thereof was 1.0.

### <Image Formation, and Droplet Jetting Method and Conditions>

With the cyan pigment ink C, magenta pigment ink M, yellow pigment ink Y, black pigment ink K and treatment solution, by use of a unit shown in Fig. 3, under the conditions below, a 4 color single pulse image was formed. At that time, a grey scale and a character image were formed.

### -Treatment Solution Head for Pre-coat Module-

Head: 600 dots per 2.54 cm/0.51 m (600 dpi/20 inch) width piezo full-line head
Amount of discharge droplet: two-values recording of 0, 4.0 pL
Drive frequency: 15 kHz (conveying speed of recording medium: 635 mm/sec)
Image drawing pattern: a pattern that imparts, in the ink drawing step, a treatment solution in advance to positions where color ink of at least one color is drawn is applied.

### ~Water Drying (Air Blow Drying) for Pre-coat Module

Speed of wind: 15 m/sec
Temperature: a contact planar heater was used to heat from a back surface of a recording surface of a recording medium so that a surface temperature of the recording medium may be 60°C
Air blowing region: 450 mm (drying time: 0.7 sec)

### -Ink Drawing-

Head: a 1,200 dots per 2.54 cm/0.51 m (1,200 dpi/20 inch) width piezo full-line head was disposed for each of four colors
Amount of discharge droplet: four-values recording of 0, 2.0, 3.5, 4.0 pL
Drive frequency: 30 kHz (conveying speed of recording medium: 635 mm/sec)

### -Drying (water drying, air blow drying)-

Speed of wind: 15 m/s
Temperature: 60°C
Air blow region: 640 mm (drying time: 1 sec)

### -Heating and Fixing-

Silicone rubber roller (hardness: 50°, nip width: 5 mm)
Roller temperature: 90°C
Pressure: 0.8 MPa

Subsequently, the following evaluation 4 and a tape peeling test were performed.

### -4. Evaluation of jetted droplet-

The gray scale and character images which were formed above were visually observed, and then evaluated according to the following evaluation criteria. The evaluation results are shows, in Table 1.

### <Evaluation criteria>

A: No image blur and no mixing of colors were observed, and the Chinese Character " " (hawk) of 4 pt or lower was resolved.
B: No image blur and no mixing of colors were observed, and the Chinese Character " " (hawk) up to 5 pt was resolved.
C: Image blur and mixing of colors were observed at many portions, and practicability was low.
D: Image blur and mixing of colors were remarkably observed at many portions, and practicability was extremely low.

### - 5. Tape peeling test -

3 hours after fixation, a 12 mm wide mending tape (manufactured by 3M. company) was stuck to a printed part. Thereafter, the peeling degree of the printed part at the time when the tape was peeled from the printed part was visually evaluated according to the following criteria. The evaluation results are shown in Table 1.
A: Peeling of the printed part was not observed.
B: Peeling of the printed part was observed, but little or no influence was observed in the image on the paper.
C: Peeling of the printed part was observed, and the image on the paper partially remained.
D: Peeling of the printed part was remarkable, and almost no image remained on the paper.

### (Example 2)

An ink jet recording medium was produced and evaluated in a manner substantially similarly to in Example 1, expect changing PVA245 of Example 1 to PVA235. The evaluation results are shown in Table 1.

### (Example 3)

An ink jet recording medium was produced and evaluated in a manner substantially similarly to in Example 1, expect changing PVA245 of Example 1 to PVA220. The evaluation results are shown in Table 1.

### (Example 4)

An inkjet recording medium was produced and evaluated in a manner substantially similarly to in Example 1, expect changing Kaobright 90 of Example 1 to Kao gloss 90 (Shiraishi Calcium Kaisha, Ltd.). The evaluation results are shown in Table 1.

### (Example 5)

An ink jet recording medium was produced and evaluated in a manner substantially similarly to in Example 1, expect changing Kaobright 90 of Example 1 to Kaolux HS (Shiraishi Calcium Kaisha, Ltd.). The evaluation results are shown in Table 1.

### (Example 6)

An ink jet recording medium was produced and evaluated in a manner substantially similarly to in Example 1, expect changing PVA245 of Example I to PVA145. The evaluation results are shown in Table 1.

### (Example 7)

An ink jet recording medium was produced and evaluated in a manner substantially similarly to in Example 1, expect changing 100 parts of 22.5% polyester urethane latex water dispersion of Example 1 to 64 parts of 35% acrylic latex water dispersion (Glass transition temperature: 60°C; Minimum film forming temperature: 50°C; Tradename: Aquabrid 4635, manufactured by Daicel Chemical Industries, Ltd.). The evaluation results are shown in Table 1.

### (Example 8)

An ink jet recording medium was produced and evaluated in a manner substantially similarly to in Example 1, expect changing PVA245 of Example to PVA210. The evaluation results are shown in Table 1.

### (Example 9)

An ink jet recording medium was produced and evaluated in a manner substantially similarly to in Example 1, expect changing PVA245 of Example 1 to PVA420. The evaluation results are shown in Table 1.

### (Comparative Example 1)

An ink jet recording medium was produced and evaluated in a manner substantially similarly to in Example 1, expect changing 100 parts of 7% aqueous PVA245 solution (manufactured by Kuraray) to 14.6 parts of 48% styrene-butadiene copolymer latex (Tradename: SN-307, manufactured by Japanese A and L Co., Ltd.). The evaluation results are shown in Table 1.

### (Comparative Example 2)

An ink jet recording medium was produced and evaluated in a manner substantially similarly to in Example 1, expect changing Kaoblight 90 to titanium oxide (Tradename: TIPAQUE R280, manufactured by Ishihara Sangyo Kaisha, Ltd.). The evaluation results are shown in Table 1.

### (Comparative Example 3)

An ink jet recording medium was produced and evaluated in a manner substantially similarly to in Example 1, expect changing 100 parts of Kaoblight 90 to 20 parts of titanium oxide (Tradename: TIPAQUE R280, manufactured by Ishihara Sangyo Kaisha, Ltd.) and 80 parts of calcium carbonate (Tradename: Escaron #2000, manufactured by Sankyo Seifun Co. Ltd.). The evaluation results are shown in Table 1.

### (Comparative Example 4)

An ink jet recording medium was produced and evaluated in a manner substantially similarly to in Example 1, expect changing Kaobright 90 of Example 10 to calcined kaolin (manufactured by Shiraishi Calcium Kaisha, Ltd.). The evaluation results are shown in Table 1.

### (Comparative Example 5)

An ink jet recording medium was produced and evaluated in a manner substantially similarly to in Example 1, expect the first layer was not formed. The evaluation results are shown in Table 1.

### (Comparative Example 6)

An ink jet recording medium was produced and evaluated in a manner substantially similarly to in Example 1, expect changing the application amount at the time of forming the first layer of Example 1 to 4 g/m². The evaluation results are shown in Table 1.

### (Comparative Example 7)

An ink jet recording medium was produced and evaluated in a manner substantially similarly to in Example 1, expect changing the application amount at the time of forming the second layer of Example 1 to 10 g/m². The evaluation results are shown in Table 1.

**[Table 1]**

| | First Layer | Second Layer | | | Evaluation | | | | |
|---|---|---|---|---|---|---|---|---|---|
| | | Kaolin | PVA | Other Additives | Water absoption amount (Bristow) (mL/m2) | Cobb water absorpt ion degree (g/m²) | Jetted droplet test | Curl test | Tape peelability |
| Example 1 | Urethane | Kaobright 90 | PVA245 | none | 3.7 | 0.9 | A | A | A |
| Example 2 | Urethane | Kaobright 90 | PVA235 | none | 3.8 | 0.9 | A | A | A |
| Example 3 | Urethane | Kaobright 90 | PVA220 | none | 3.6 | 0.9 | A | A | A |
| Example 4 | Urethane | Kaogloss 90 | PVA245 | none | 3.7 | 0.9 | A | A | A |
| Example 5 | Urethane | KaoLux HS | PVA245 | none | 3.6 | 0.9 | A | A | A |
| Example 6 | Urethane | Kaobright 90 | PVA145 | none | 3.9 | 0.9 | A | A | A |
| Example 7 | Acrylic | Kaobright 90 | PVA245 | none | 3.6 | 0.9 | A | A | A |
| Example 8 | Urethane | Kaobright 90 | PVA210 | none | 3.8 | 0.9 | A | A | B |
| Example 9 | Urethane | Kaobright 90 | PVA420 | none | 3.7 | 0.9 | A | A | B |
| Comparative Example 1 | Urethane | Kaobright 90 | none | SBR | 3.4 | 0.9 | A | A | C |
| Comparative Example 2 | Urethane | none | PVA245 | Titanium oxide | 10.8 | 0.9 | A | A | D |
| Comparative Example 3 | Urethane | none | PVA245 | Calcium carbonate +Titanium oxide | 8.5 | 0.9 | C | A | C |
| Comparative Example 4 | Urethane | Calcined kaolin | PVA245 | none | 10.2 | 0.9 | A | A | D |
| Comparative Example 5 | none | Kaobright 90 | PVA245 | none | 3.7 | - | A | C | A |
| Comparative Example 6 | Application Amount 4 g/m² | Kaobright 90 | PVA245 | none | 3.9 | 4.8 | A | C | A |
| Comparative Example 7 | Urethane | Kaobright 90 | PVA245 | Application Amount 10 g/m² | 1.8 | 0.9 | C | A | A |

As shown in the table 1, in Examples 1 to 9 in which the Cobb water absorption degree during a contact time of 120 seconds by a water absorption test according to JIS P8140 was adjusted to 2.0 g/m² or lower and also the water absorption amount during a contact time 0.5 second by Bristow method of the second layer was adjusted to from 2 mL/m² to 8 mL/m², no problems occurred in all the jetted droplet test, curl test, and tape peeling test. Especially in Examples 1 to 7, the best evaluation results were obtained in all the items. In contrast, in Comparative Examples 1 to 7, problems occurred in at least one of the jetted droplet test, curl test, and tape peeling test.

The present invention can provide a recording medium which can form a high quality image in which the development of curl, image blur, and mixing of colors occurring in connection with image recording are prevented and separation of ink is difficult to occur; a method of producing the same; and an ink jet recording method which allows formation of a high quality image at low cost and at high speed.

The foregoing description of the exemplary embodiments of the present invention has been provided for the purposes of illustration and description. It is not intended to be exhaustive or to limit the invention to the precise forms disclosed. The embodiments were chosen and described in order to best explain the principles of the invention and its practical applications, thereby enabling others skilled in the art to understand the invention for various embodiments and with the various modifications as are suited to the particular use contemplated. It will be obvious to those having skill in the art that many changes may be made in the above-described details of the preferred embodiments of the present invention. It is intended that the scope of the invention be defined by the following claims.

## Claims

1. A recording medium (100), comprising:
a base paper (11),
a first layer (12) containing a binder, and
a second layer (13) containing kaolin and Polyvinyl alcohol,
the base paper (11), the first layer (12), and the second layer (13) being successively laminated, wherein
a Cobb water absorption degree during a contact time of 120 seconds by a water absorption test according to JIS P8140 on the surface of the first layer (12) formed on the base paper (11) on which the first layer (12) has been formed is 2.0 g/m2 or less; and
the water absorption amount during a contact time of 0.5 second by the Bristow method on the surface of the second layer (13) is from 2 mL/m2 to 8 mL/m2,
wherein the kaolin has a whiteness degree of more than 87 and the composition ratio (volume ratio) of kaolin having a particle diameter of 2 µm or less is 75% or more with respect to a total volume of kaolin, and wherein the degree of polymerization of the polyvinyl alcohol is 1500 or more.

2. The recording medium (100) of Claim 1, wherein the content of the kaolin in the second layer (13) is from 75% by mass to 99% by mass with respect to the total solid content of the second layer (13).

3. The recording medium (100) of any one of Claim 1 to 2, wherein the binder in the first layer (12) contains a thermoplastic resin.

4. The recording medium (100) of claim 3, wherein the thermoplastic resin is at least one selected from the group consisting of polyester urethane latex and acrylic silicone latex.

5. The recording medium (100) of any one of Claim 1 to 4, wherein the first layer (12) further contains a white pigment.

6. The recording medium (100) of Claim 5, wherein the white pigment is kaolin.

7. A method of producing of the recording medium (100) of any one of Claim 3 to 6, the method comprising:
forming a first layer (12) on a base paper (11) by applying a film formation liquid containing a thermoplastic resin particle, and heating at a temperature range equal to or higher than the minimum film forming temperature of the thermoplastic resin particle; and
forming a second layer (13) on the first layer (12) by applying a film formation liquid containing kaolin and polyvinyl alcohol to the first layer (12).

8. An ink jet recording method, comprising:
applying ink to the recording medium (100) of any one of Claim 1 to 6, and performing ink drawing according to predetermined image data, and
drying and removing an ink solvent in the recording medium (100) on which ink drawing has been performed.

9. An ink jet recording method, comprising:
applying a treatment liquid containing an acid substance to the recording medium (100) of any one of Claim 1 to 6;
applying ink to the recording medium (100) to which the treatment liquid has been applied, and performing ink drawing according to predetermined image data; and
drying and removing an ink solvent in the recording medium (100) on which ink drawing has been performed.

## Patentansprüche

1. Aufzeichnungsmedium (100), umfassend:
ein Basispapier (11),
eine erste Schicht (12), die ein Bindemittel enthält, und
eine zweite Schicht (13), die Kaolin und Polyvinylalkohol enthält,
wobei das Basispapier (11), die erste Schicht (12) und die zweite Schicht (13) sukzessive laminiert sind, worin
der Cobb-Wasserabsorptionsgrad während einer Kontaktzeit von 120 Sekunden mit einem Wasser-Absorptionstest gemäß JIS P8140 auf der Oberfläche der ersten Schicht (12), gebildet auf dem Basispapier (11), auf dem die erste Schicht (12) gebildet worden ist, 2,0 g/m² oder weniger beträgt; und
die Wasserabsorptionsmenge während einer Kontaktzeit von 0,5 Sekunden mit dem Bristow-Verfahren auf der Oberfläche der zweiten Schicht (13) 2 ml/m² bis 8 ml/m² beträgt,
worin das Kaolin einen Weißgrad von mehr als 87 aufweist und das Zusammensetzungsverhältnis (Volumenverhältnis) von Kaolin mit einem Partikeldurchmesser von 2 µm oder kleiner 75 % oder mehr in Bezug auf das Gesamtvolumen von Kaolin beträgt, und worin der Polymerisationsgrad des Polyvinylalkohols 1.500 oder größer ist.

2. Aufzeichnungsmedium (100) gemäß Anspruch 1, worin der Kaolingehalt in der zweiten Schicht (13) 75 bis 99 Masse% beträgt, bezogen auf den Gesamtfeststoffgehalt der zweiten Schicht (13).

3. Aufzeichnungsmedium (100) gemäß irgendeinem der Ansprüche 1 bis 2, worin das Bindemittel in der ersten Schicht (12) ein thermoplastisches Harz enthält.

4. Aufzeichnungsmedium (100) gemäß Anspruch 3, worin das thermoplastische Harz mindestens eines ist, ausgewählt aus der Gruppe bestehend aus Polyesterurethanlatex und Acrylsilikonlatex.

5. Aufzeichnungsmedium (100) gemäß irgendeinem der Ansprüche 1 bis 4, worin die erste Schicht (12) ferner ein weißes Pigment enthält.

6. Aufzeichnungsmedium (100) gemäß Anspruch 5, worin das weiße Pigment Kaolin ist.

7. Verfahren zur Herstellung des Aufzeichnungsmediums (100) gemäß irgendeinem der Ansprüche 3 bis 6, wobei das Verfahren umfasst:
Bilden einer ersten Schicht (12) auf einem Basispapier (11) durch Auftragen einer Filmbildungsflüssigkeit, die thermoplastische Harzpartikel enthält, und Erwärmen in einem Temperaturbereich, der gleich oder höher ist als die minimale Filmbildungstemperatur der thermoplastischen Harzpartikel; und
Bilden einer zweiten Schicht (13) auf der ersten Schicht (12) durch Auftragen einer Filmbildungsflüssigkeit, die Kaolin und Polyvinylalkohol enthält, auf die erste Schicht (12).

8. Tintenstrahl-Aufzeichnungsverfahren, umfassend:
Auftragen von Tinte auf das Aufzeichnungsmedium (100) gemäß irgendeinem der Ansprüche 1 bis 6 und Durchführen einer Tintenzeichnung gemäß vorbestimmten Bilddaten, und
Trocknen und Entfernen eines Tintenlösungsmittels in dem Aufzeichnungsmedium (100), auf dem das Tintenzeichnen durchgeführt worden ist.

9. Tintenstrahl-Aufzeichnungsverfahren, umfassend:
Auftragen einer Behandlungsflüssigkeit, die eine saure Substanz enthält, auf das Aufzeichnungsmedium (100) gemäß irgendeinem der Ansprüche 1 bis 6;
Auftragen von Tinte auf das Aufzeichnungsmedium (100), auf das die Behandlungsflüssigkeit aufgetragen worden ist, und Durchführen von Tintenzeichnen gemäß vorbestimmten Bilddaten; und
Trocknen und Entfernen eines Tintenlösungsmittels in dem Aufzeichnungsmedium (100), auf dem das Tintenzeichnen durchgeführt worden ist.

## Revendications

1. Support d'enregistrement (100), comprenant :
un papier de base (11),
une première couche (12) contenant un liant, et
une seconde couche (13) contenant du kaolin et de l'alcool de polyvinyle,
le papier de base (11), la première couche (12) et la seconde couche (13) étant stratifiés en succession, dans lequel
un degré Cobb d'absorption d'eau pendant un temps de contact de 120 secondes par un test d'absorption d'eau selon JIS P8140 sur la surface de la première couche (12) formée sur le papier de base (11) sur lequel la première couche (12) a été formée est de 2,0 g/m² ou moins ; et
la quantité d'absorption d'eau pendant un temps de contact de 0,5 seconde par le procédé Bristow sur la surface de la seconde couche (13) est de 2 ml/m² à 8 ml/m²,
dans lequel le kaolin a un degré de blancheur supérieur à 87 et le rapport de composition (rapport de volume) du kaolin ayant un diamètre de particule de 2 µm ou moins est de 75 % ou plus par rapport à un volume total de kaolin, et dans lequel le degré de polymérisation de l'alcool de polyvinyle est de 1 500 ou plus.

2. Support d'enregistrement (100) selon la revendication 1, dans lequel la teneur en kaolin dans la seconde couche (13) est de 75 % en masse à 99 % en masse par rapport à la teneur totale en solides de la seconde couche (13).

3. Support d'enregistrement (100) selon l'une quelconque des revendications 1 à 2, dans lequel le liant dans la première couche (12) contient une résine thermoplastique.

4. Support d'enregistrement (100) selon la revendication 3, dans lequel la résine thermoplastique est au moins une sélectionnée à partir du groupe constitué par le latex de polyesteruréthane et le latex de silicone acrylique.

5. Support d'enregistrement (100) selon l'une quelconque des revendications 1 à 4, dans lequel la première couche (12) contient en outre un pigment blanc.

6. Support d'enregistrement (100) selon la revendication 5, dans lequel le pigment blanc est du kaolin.

7. Procédé de production du support d'enregistrement (100) selon l'une quelconque des revendications 3 à 6, le procédé comprenant :
la formation d'une première couche (12) sur un papier de base (11) en appliquant un liquide de formation de film contenant une particule de résine thermoplastique, et le chauffage à une plage de températures égale ou supérieure à la température minimale de formation de film de la particule de résine thermoplastique ; et
la formation d'une seconde couche (13) sur la première couche (12) en appliquant un liquide de formation de film contenant du kaolin et de l'alcool de polyvinyle à la première couche (12).

8. Procédé d'enregistrement à jet d'encre, comprenant :
l'application d'encre au support d'enregistrement (100) selon l'une quelconque des revendications 1 à 6, et l'exécution d'un tracé à l'encre selon des données d'image prédéterminées, et
le séchage et l'enlèvement d'un solvant d'encre dans le support d'enregistrement (100) sur lequel un tracé à l'encre a été effectué.

9. Procédé d'enregistrement à jet d'encre, comprenant :
l'application d'un liquide de traitement contenant une substance acide au support d'enregistrement (100) selon l'une quelconque des revendications 1 à 6 ;
l'application d'encre au support d'enregistrement (100) auquel le liquide de traitement a été appliqué, et l'exécution d'un tracé à l'encre selon des données d'image prédéterminées ; et
le séchage et l'enlèvement d'un solvant d'encre dans le support d'enregistrement (100) sur lequel un tracé à l'encre a été effectué.
